



US006248483B1

(12) **United States Patent**  
Aylward et al.

(10) **Patent No.:** US 6,248,483 B1  
(45) **Date of Patent:** Jun. 19, 2001

(54) **PAPER BASE TRANSMISSION DISPLAY MATERIAL**

(75) Inventors: **Peter T. Aylward**, Hilton; **Alphonse D. Camp**, Rochester; **Robert P. Bourdelais**, Pittsford; **Geoffrey Mruk**, Rochester, all of NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/552,130**

(22) Filed: **Apr. 19, 2000**

(51) **Int. Cl.<sup>7</sup>** G03C 1/765; G03C 1/785; G03C 1/79; G03C 11/08

(52) **U.S. Cl.** 430/12; 430/432; 430/201; 430/496; 430/527; 430/536; 430/538; 430/961; 430/14

(58) **Field of Search** 430/536, 538, 430/496, 12, 527, 961, 432, 201, 14; 347/106

(56)

**References Cited**

**U.S. PATENT DOCUMENTS**

|           |   |        |                        |         |
|-----------|---|--------|------------------------|---------|
| 5,212,053 | * | 5/1993 | McSweeney et al. ....  | 430/538 |
| 5,212,503 |   | 5/1993 | Saito et al. ....      | 346/140 |
| 5,866,282 |   | 2/1999 | Bourdelaïs et al. .... | 430/536 |
| 5,888,681 |   | 3/1999 | Gula et al. ....       | 430/536 |
| 6,017,686 |   | 1/2000 | Aylward et al. ....    | 430/536 |
| 6,030,742 |   | 2/2000 | Bourdelaïs et al. .... | 430/536 |
| 6,071,654 |   | 6/2000 | Camp et al. ....       | 430/536 |
| 6,083,669 |   | 7/2000 | Bourdelaïs et al. .... | 430/533 |

\* cited by examiner

*Primary Examiner*—Richard L. Schilling

(74) *Attorney, Agent, or Firm*—Paul A. Leipold

**ABSTRACT**

The invention relates to a transmission display material comprising a paper base, a lower layer of biaxially oriented polymer sheet, a polyethylene layer on the upper side of said paper base, and at least one image layer overlaying said polyethylene layer.

**24 Claims, No Drawings**

## PAPER BASE TRANSMISSION DISPLAY MATERIAL

### FIELD OF THE INVENTION

This invention relates to imaging materials. In a preferred form it relates to base materials for imaging translucent paper display.

### BACKGROUND OF THE INVENTION

It is known in the art that photographic display materials are utilized for advertising, as well as decorative displays of photographic images. Since these display materials are used in advertising, the image quality of the display material is critical in expressing the quality message of the product or service being advertised. Further, a photographic display image needs to be high impact, as it attempts to draw consumer attention to the display material and the desired message being conveyed. Typical applications for display material include product and service advertising in public places such as airports, buses and sports stadiums, movie posters, point of purchase areas such as store fronts, illuminate billboards and fine art photography. The desired attributes of a quality, high impact photographic display material are a slight blue density minimum, durability, sharpness, and flatness. Cost is also important, as display materials tend to be expensive compared with alternative display material technology, mainly lithographic images on paper. For display materials, traditional color paper is undesirable, as it suffers from a lack of durability for the handling, photoprocessing, and display of large format images.

In the formation of color paper it is known that the base paper has applied thereto a layer of polymer, typically polyethylene. This layer serves to provide waterproofing to the paper, as well as providing a smooth surface on which the photosensitive layers are formed. The formation of a suitably smooth surface is difficult, requiring great care and expense to ensure proper laydown and cooling of the polyethylene layers. The formation of a suitably smooth surface would also improve image quality, as the display material would have more apparent blackness as the reflective properties of the improved base are more specular than the prior materials. As the whites are whiter and the blacks are blacker, there is more range in between and, therefore, contrast is enhanced. It would be desirable if a more reliable and improved surface could be formed at less expense.

Prior art photographic transmission display materials with incorporated diffusers have light sensitive silver halide emulsions coated directly onto a gelatin coated clear polyester sheet. Incorporated diffusers are necessary to diffuse the light source used to illuminate transmission display materials. Without a diffuser, the light source would reduce the quality of the image. Typically, white pigments are coated in the bottom most layer of the imaging layers. Since light sensitive silver halide emulsions tend to be yellow because of the gelatin used as a binder for photographic emulsions, minimum density areas of a developed image will tend to appear yellow. A yellow density minimum reduces the commercial value of a transmission display material because the imaging viewing public associates image quality with a white density minimum. It would be desirable if a transmission display material with an incorporated diffuser could have a more blue density minimum which people perceptually prefer.

It has been proposed in U.S. Pat. No. 5,212,053 to use a cellulose paper base with a basis weight less than 120 g/m<sup>2</sup>

as a support for a photographic translucent display material. In U.S. Pat. No. 5,212,053 numerous advantages are obtained by the use of cellulose paper as a base. Advantages such as the low cost of paper compared to suitable polymer bases and an increase in manufacturing efficiency gained by the use of color photographic paper forming apparatus were disclosed. While all of these improvements are possible with the use of a melt cast extruded polyethylene paper base, the paper base does not have the required strength properties to be reliability processed in wet chemistry common with the imaging development process.

Typically transmission display materials require more saturated colors so they appear as true colors to the viewer. In a photographic system, it is common to coat up 2 to 2.5 times the normal coverage of a reflection print. This added coverage contains gelatin. When gelatin is dried after the processing operation, there is a large force exerted on the base because of the shrinkage forces within the gelatin structure. On melt cast polyethylene paper, this force can cause the paper imaging element to curl excessively and crease making the element unusable. When the illuminated photographic display materials are processed utilizing weak paper and low strength polyethylene layers, the web can break causing a loss in efficiency in commercial photoprocessing labs. Further, the thin papers disclosed in U.S. Pat. No. 5,212,053 are not strong enough for efficient transport in digital printing equipment such as ink jet printers or thermal dye transfer printers. It would be desirable if translucent display material with a cellulose paper base had the required strength properties for efficient transport through digital printers, yet was thin enough to exhibit the required transmission properties. The paper disclosed in U.S. Pat. No. 5,212,053, while providing a good display material when coated with a gelatin based silver halide photographic emulsion and placed in a low relative humidity environment, has a tendency to curl towards the image side. This may create some difficulties during mounting of this display material. Excessive curl can cause problems in handling and constraining the display material which may cause damage and distract from its commercial value. It would be desirable to have a paper base transmission material that has less curl and handles better than prior art materials.

Prior art photographic transmission display materials with incorporated diffusers have light sensitive silver halide emulsions coated directly onto a gelatin subbed clear polyester sheet. TiO<sub>2</sub> is added to the bottom most layer of the imaging layers to diffuse light so that individual elements of the illuminating bulbs utilized are not visible to the observer of the displayed image. However, coating TiO<sub>2</sub> in the imaging layer causes manufacturing problems such as increased coating coverage which requires more coating machine drying and a reduction in coating machine productivity as the TiO<sub>2</sub> requires additional cleaning of the coating machine. Further, as higher amounts of TiO<sub>2</sub> are used to diffuse high intensity illumination systems, the TiO<sub>2</sub> coated in the bottom most imaging layer causes unacceptable light scattering reducing the quality of the transmission image. It would be desirable to reduce or eliminate the TiO<sub>2</sub> from the image layers while providing the necessary transmission properties and image quality properties.

Prior art photographic transmission display material use polyester as a base for the support. Typically the polyester support is from 150 to 250  $\mu\text{m}$  thick to provide the required stiffness. A cellulose paper base material would be lower in cost and allow for roll handling efficiency, as the rolls would weigh less and be smaller in diameter. It would be desirable to use a low cost base material that had the required stiffness but was thinner to reduce cost and improve roll handling efficiency.

Prior art photographic transmission display materials, while providing excellent image quality, tend to be expensive when compared with other quality imaging technologies such as ink jet imaging, thermal dye transfer imaging, and gravure printing. Since photographic transmission display materials require an additional imaging processing step compared to digital imaging systems such as ink jet printing and thermal dye transfer printing, the cost of a transmission photographic display can be higher than digital imaging systems. The processing equipment investment required to process photographic transmission display materials also requires consumers to typically interface with a commercial processing lab, increasing time required to move from concept to image. It would be desirable if a high quality transmission display support could utilize nonphotographic quality imaging technologies.

Photographic transmission display materials have considerable consumer appeal as they allow images to be printed on high quality support for home or small business use. Consumer use of photographic display materials generally have been cost prohibitive since consumers typically do not have the required volume to justify the use of such materials. It would be desirable if a high quality transmission display material could be used in the home without a significant investment in equipment to print the image

#### PROBLEM TO BE SOLVED BY THE INVENTION

There is a need for low cost paper transmission display materials that provide improved transmission of light while, at the same time, more efficiently diffusing the illuminating light source such that the elements of the illuminating light source are not apparent to the viewer.

#### SUMMARY OF THE INVENTION

It is an object of the invention to provide improved transmission display materials.

It is another object to provide display materials that are lower in cost, as well as providing sharp durable images.

It is a further object to provide more efficient use of the light used to illuminate transmission display materials.

It is another object to provide a thin imaging base with the required strength properties to ensure more efficient handling and display of images.

It is further object to provide a transmission display that utilizes non photographic imaging technology.

It is an additional object to provide a transmission display that utilizes photographic imaging technology.

These and other objects of the invention are accomplished by a transmission display material comprising a paper base, a lower layer of biaxially oriented polymer sheet, a polyethylene layer on the upper side of said paper base, and at least one image layer overlaying said polyethylene layer.

#### ADVANTAGEOUS EFFECT OF THE INVENTION

The invention provides a low cost support with brighter images by allowing more efficient diffusion of light used to illuminate display materials. The support will control the diffusing of light predominately by the paper base. By utilizing a biaxially oriented sheet on the backside and pre-stressing the base prior to emulsion coating, the imaging element can overcome creasing problems making this invention more desirable.

#### DETAILED DESCRIPTION OF THE INVENTION

The invention has numerous advantages over prior transmission display materials and methods of imaging transmis-

sion display materials. The display materials of the invention provide very efficient diffusing of light while allowing the transmission of a high percentage of the light. The materials are low in cost, as the translucent cellulose paper base is thinner than in prior products, yet strong enough to provide improved handling and display of images. The formation of transmission display materials requires a display material that diffuses light so well that individual elements of the illuminating bulbs utilized are not visible to the observer of the displayed image. On the other hand, it is necessary that light be transmitted efficiently to brightly illuminate the display image. The invention allows a greater amount of illuminating light to actually be utilized as display illumination while, at the same time, very effectively diffusing the light sources such that they are not apparent to the observer.

Because this display material may be used with either photographic or nonphotographic imaging layers, the display material has substantial appeal to the consumer, as digital printing systems such as ink jet or thermal dye transfer are widely available and low in cost for small volume or in the case of a photofinisher who has an existing photographic system may select a display material containing a silver halide imaging layer. This allows the consumer to select a display material that best fits their equipment infrastructure. This flexibility allows the consumer to optimize their business not only on image quality but also capital investment or even environmental problems associated with the use and disposal of processing chemicals. A further advantage of the invention is the ability to provide non glossy surfaces to the imaging element. Currently, glossy display material have applied to the surface, a matte coating which reduces the gloss of the image. By providing a non glossy support material, there is no need for post process application of a expensive matte surface. These and other advantages will be apparent from the detailed description below.

The terms as used herein, "top", "upper", "imaging side", and "face" mean the side or toward the side of the display material with the imaging layer. The terms "bottom", "lower side", and "back" mean the side opposite or toward the side opposite of the imaging layer. The term as used herein, "transparent" means the ability to pass radiation without significant deviation or absorption. For this invention, "transparent" material is defined as a material that has a spectral transmission greater than 90%. For an imaging element, spectral transmission is the ratio of the transmitted power to the incident power and is expressed as a percentage as follow;  $T_{RGB}=10^{-D}*100$  where D is the average of the red, green and blue Status A transmission density response measured by an X-Rite Model (310) (or comparable) photographic transmission densitometer.

The transmission display material of this invention comprises a paper base, a lower layer of biaxially oriented polymer sheet, a polyethylene layer on the upper side of said paper base, and at least one image layer overlaying said polyethylene layer. The said image layer of said transmission display material of this invention may comprise at least one silver halide containing layer or at least one ink jet receiving layer. Since the display material substrate can be coated either with a silver halide containing layer or an ink jet receiving layer, there is added flexibility and economy by only having a single substrate that can be used with varying imaging technology. The layers of the biaxially oriented polyolefin sheet of this invention are substantially free of voids,  $TiO_2$  and colorants because the biaxially oriented polyolefin sheet comprises the side opposite to the imaging side. In this case the optimum transmission properties are

substantially controlled by a low cost cellulose paper base. There is a thin layer of a pigmented polyethylene polymer comprising the top layer in direct contact with the silver halide emulsion containing layers. In this case the layer comprising polymer and  $TiO_2$  improves the image sharpness because the paper is imaged with an optical exposure. The layer is of sufficient thinnest and concentration of white pigment such that it does not substantially effect the total transmission properties of the display material. Further, because a thin layer of polyolefin is cast coated on the surface of the paper, the surface roughness of the cast coated polyolefin sheet can increased to provide a non glossy surface. A non-glossy surface has significant commercial value in that the common practice of post process application of a matte coating could be eliminated.

The transmission display material of this invention has a spectral transmission of between 30 and 70 percent but in the most preferred case has a spectral transmission of between 40 and 60 percent. A spectral transmission of between 40 and 60 percent is preferred because it provides the optimum level of light transmission that provides a clear, sharp, snappy display image that is eye catching while also providing sufficient opacity to hide the illuminating. Spectral transmission is the amount of light energy that is transmitted through a material. For an imaging element, spectral transmission is the ratio of the transmitted power to the incident power and is expressed as a percentage as follows:  $T_{RGB} = 10^{-D} * 100$  where D is the average of the red, green, and blue Status A transmission density response measured by an X-Rite model 310 (or comparable) photographic transmission densitometer. The higher the transmission, the less opaque the material. For a transmission display material with an incorporated diffuser, the quality of the image is related to the amount of light reflected from the image to the observer's eye. A transmission display image with a low amount of spectral transmission does not allow sufficient illumination of the image causing a perceptual loss in image quality. A transmission image with a spectral transmission of less than 30% is unacceptable for a transmission display material, as the quality of the image cannot match prior art transmission display materials. Further, spectral transmissions less than 30% will require additional dye density which increases the cost of the transmission display material.

The paper provides an efficient means of diffusing the illuminating light source used to illuminate the image. The many cellulose paper fiber/air interfaces in the cellulose paper of this invention diffuse the illuminating light without interfering with the quality of the image. Paper fiber is also lower in cost than a polymer base making cellulose paper a very good low cost transmission display base material. Thin paper bases are utilized in this invention and are much thinner than conventional paper bases used in reflective images. Paper bases used in reflective print materials are typically several times thicker than the paper bases used in this invention. A thick reflective paper base is not suitable for this invention because the low light transmission of a reflective paper base would not allow for sufficient illumination of the image. The preferred transmission display material comprising a paper base, a lower biaxially oriented sheet, a polyethylene layer on the upper side of said paper base, and at least one imaging layer overlaying said polyethylene layer. The paper base has a basis weight of between 50 and 150 g/m<sup>2</sup> and an apparent density of between 0.97 g/cc and 1.2 g/cc. The transmission display material has a tensile strength of between 20,400 kPa and 68,000 kPa. The basis weight of said paper base provides sufficient opacity to

allow the filaments or light bulb in the display box to be hidden while allowing adequate light to be transmitted through the image to provide a very eye-catching image. Paper used in this invention is selected to have a uniform formation allowing light to be transmitted with minimal paper structure visible.

The paper used in this invention comprises cellulose fiber that have been refined and pressed into a uniform sheet of paper. Any pulps known in the art to provide image quality paper may be used in this invention. Bleached hardwood chemical kraft pulp is preferred, as it provides brightness, a good starting surface, and good formation while maintaining strength. In general, hardwood fibers are much shorter than softwood by approximately a 1:3 ratio. Pulp with a brightness less than 90% brightness at 457 nm is preferred. Pulps with brightness of 90% or greater are commonly used in imaging supports because consumers typically prefer a white paper appearance. A cellulose paper less than 90% brightness at 457 nm is preferred for cost reasons, as the whiteness of the imaging support can be improved by laminating a microvoided biaxially oriented sheet to the cellulose paper of this invention. The reduction in brightness of the pulp allows for a reduction in the amount of bleaching required, thus lowering the cost of the pulp and reducing the bleaching load on the environment.

Cellulose paper used in this invention can be made on a standard continuous fourdrinier wire machine. For the formation of cellulose paper of this invention, it is necessary to refine the paper fibers to a high degree to obtain good formation. This may be accomplished in this invention by providing wood fibers suspended in water, bringing said fibers into contact with a series of disc refining mixers and conical refining mixers such that fiber development in disc refining is carried out at a total specific net refining power of 44 to 66 KW hrs/metric ton and cutting in the conical mixers is carried out at a total specific net refining power of between 55 and 88 KW hrs/metric ton, applying said fibers in water to a foraminous member to remove water, drying said paper between press and felt, drying said paper between cans, applying a size to said paper, drying said paper between steam heated dryer cans, applying steam to said paper, and passing said paper through calender rolls. The preferred specific net refining power (SNRP) of cutting is between 66 and 77 KW hrs/metric ton. A SNRP of less than 66 KW hrs/metric ton will provide an inadequate fiber length reduction resulting in a less smooth surface. A SNRP of greater than 77 KW hrs/metric ton after disc refining described above generates a stock slurry that is difficult to drain from the fourdrinier wire. Specific Net Refiner Power is calculated by the following formula: (Applied Power in Kilowatts to the refiner—the No Load Kilowatts)/(0.251 \* % consistency\*flow rate in gpm\*0.907 metric tons/ton).

For the formation of cellulose paper of sufficient smoothness, it is desirable to rewet the paper surface prior to final calendering. Papers made on the paper machine with a high moisture content calendar much more readily than papers of the same moisture content containing water added in a remoistening operation. This is due to a partial irreversibility in the imbibition of water by cellulose. However, calendering a paper with high moisture content results in blackening, a condition of transparency resulting from fibers being crushed in contact with each other. The crushed areas reflect less light and, therefore, appear dark, a condition that is undesirable in an imaging application such as a base for imaging materials. By adding moisture to the surface of the paper after, the paper has been machine dried and the problem of blackening can be avoided while preserving the

advantages of high moisture calendering. The addition of surface moisture prior to machine calendering is intended to soften the surface fibers and not the fibers in the interior of the paper. Papers calendered with a high surface moisture content generally show greater strength, density, gloss, and processing chemistry resistance, all of which are desirable for a display support and have been shown to be perceptually preferred to prior art translucent display paper bases.

There are several paper surface humidification/moisturization techniques. The application of water, either by mechanical roller or aerosol mist by way of an electrostatic field, are two techniques known in the art. The above techniques require dwell time, hence web length, for the water to penetrate the surface and equalize in the top surface of the paper. Therefore, it is difficult for these above systems to make moisture corrections without distorting, spotting, and swelling of the paper. The preferred method to rewet the paper surface prior final calendering is by use of a steam application device. A steam application device uses saturated steam in a controlled atmosphere to cause water vapor to penetrate the surface of the paper and condense. Prior to calendering, the steam application device allows a considerable improvement in gloss and smoothness due to the heating up and moisturizing the paper of this invention before the pressure nip of the calendering rolls. An example of a commercially available system that allows for controlled steam moisturization of the surface of cellulose paper is the "Fluidex System" manufacture by Pagedarm Corp. The preferred moisture content by weight after applying the steam and calendering is between 7% and 9%. A moisture level less than 7% is more costly to manufacture since more fiber is needed to reach a final basis weight. At a moisture level greater than 10%, the surface of the paper begins to degrade. After the steam foil rewetting of the paper surface, the paper is calendered before winding of the paper. The preferred temperature of the calender rolls is between 76° C. and 88° C. Lower temperatures result in a poor surface. Higher temperatures are unnecessary, as they do not improve the paper surface and require more energy. The polymer sheet of said invention should be transparent or substantially transparent so as not to interfere with the transmission of light. For the purpose of this patent transparent or substantially transparent refers to the passage of light greater than 90%. The tensile strength of the display material is important to help with the transport of material through a processing machine in the case of a photographic display material or a printer in the case of ink jet or thermal dye sublimation. The biaxially oriented polymer sheet that is used as a lower layer for the transmission display material of this invention has a surface roughness of between 0.2 and 0.8 micrometers. This roughness frequency provides good transportability through a variety of processing equipment to minimize slippage, scratching or other problems. In most case the lower most portion of the backside biaxially oriented polymer sheet further comprises an antistat layer. The antistat provides an optimum coefficient of friction to aid in good transportability as well as provides a conductive layer to allow electrostatic charges to move to a ground. This helps to prevent excessive charge buildup which if uncontrolled could lead to an electrostatic discharge that would fog a silver halide emulsion layer. In some cases an electrostatic buildup can also interfere with the ability of sheets to slide over one another without sticking.

The problem of controlling static charge is well known in the field of photography. The accumulation of charge on film or paper surfaces leads to the attraction of dirt, which can produce physical defects. The discharge of accumulated

charge during or after the application of the sensitized emulsion layer(s) can produce irregular fog patterns or "static marks" in the emulsion. The static problems have been aggravated by increase in the sensitivity of new emulsions, increase in coating machine speeds, and increase in post-coating drying efficiency. The charge generated during the coating process may accumulate during winding and unwinding operations, during transport through the coating machines and during finishing operations such as slitting and spooling.

It is generally known that electrostatic charge can be dissipated effectively by incorporating one or more electrically-conductive "antistatic" layers into the film structure. Antistatic layers can be applied to one or to both sides of the film base as subbing layers either beneath or on the side opposite to the light-sensitive silver halide emulsion layers. An antistatic layer can alternatively be applied as an outer coated layer either over the emulsion layers or on the side of the film base opposite to the emulsion layers or both. For some applications, the antistatic agent can be incorporated into the emulsion layers. Alternatively, the antistatic agent can be directly incorporated into the film base itself.

A wide variety of electrically-conductive materials can be incorporated into antistatic layers to produce a wide range of conductivity. These can be divided into two broad groups: (i) ionic conductors and (ii) electronic conductors. In ionic conductors charge is transferred by the bulk diffusion of charged species through an electrolyte. Here the resistivity of the antistatic layer is dependent on temperature and humidity. Antistatic layers containing simple inorganic salts, alkali metal salts of surfactants, ionic conductive polymers, polymeric electrolytes containing alkali metal salts, and colloidal metal oxide salts (stabilized by metal salts), described previously in patent literature, fall in this category. However, many of the inorganic salts, polymeric electrolytes, and low molecular weight surfactants used are water-soluble and are leached out of the antistatic layers during processing, resulting in a loss of antistatic function. The conductivity of antistatic layers employing an electronic conductor depends on electronic mobility rather than ionic mobility and is independent of humidity. Antistatic layers which contain conjugated polymers, semiconductive metal halide salts, semiconductive metal oxide particles, etc., have been described previously. However, these antistatic layers typically contain a high volume percentage of electronically conducting materials which are often expensive and impart unfavorable physical characteristics, such as color, increased brittleness, and poor adhesion to the antistatic layer.

Besides antistatic properties, an auxiliary layer in a photographic element maybe required to fulfill additional criteria depending on the application. For example for resin-coated photographic paper, the antistatic layer if present as an external backing layer should be able to receive prints (e.g., bar codes or other indicia containing useful information) typically administered by dot matrix printers and to retain these prints or markings as the paper undergoes processing. Most colloidal silica based antistatic backings without a polymeric binder provide poor post-processing backmark retention qualities for photographic paper. Typical antistat used in this application include a conductive agent comprises alkali metal salts of polyacids or cellulose derivatives. Other conductive agent comprises polymerized alkylene oxides and alkali metal salts. Typical binder used with these antistats may also include gelatin. Gelatin is desirable when additional reverse curl control is needed to offset high gelatin loads in the emulsion layers.

The display material comprising a paper base, a lower layer of biaxially oriented polymer sheet, a polyethylene

layer on the upper side of said paper base, and at least one image layer overlaying said polyethylene layer in the invention comprises a biaxially oriented polymer sheet further comprises a polyolefin and in the preferred case comprises a polypropylene. Polyolefin and in particular polypropylene are desirable because they provide good resistance to curl while offering a very cost efficient material. An important aspect of this invention is the high strength biaxially oriented polymer sheet laminated to the cellulose paper base. Prior art photographic cellulose paper transmission display materials suffer from a lack of strength causing problems in handling and transport through digital printers. Lamination of a high strength biaxially oriented polymer sheet to the cellulose paper not only significantly increases the strength of the imaging support, but also allows a reduction in paper thickness which improves the percent transmission of the imaging element significantly improving image quality over prior art paper transmission display materials. The biaxially oriented sheet is laminated to the bottom of the cellulose paper base only because the transmission materials of this invention may require curl control when processing and handling the material. In cases where additional curl performance is needed, materials such as polyesters may be used.

When using a cellulose paper base, it is preferable to extrusion laminate the backside composite sheets to the base paper using a polyolefin resin. Extrusion laminating is carried out by bringing together the biaxially oriented sheets of the invention and the paper base with application of a melt extruded adhesive between the paper sheets and the biaxially oriented polyolefin sheets, followed by their being pressed in a nip such as between two rollers. The melt extruded adhesive may be applied to either the biaxially oriented sheets or the base paper prior to their being brought into the nip. In a preferred form the adhesive is applied into the nip simultaneously with the biaxially oriented sheets and the base paper. The adhesive used to adhere the biaxially oriented polyolefin sheet to the paper base may be any suitable material that does not have a harmful effect upon the imaging element. A preferred material is metallocene catalyzed ethylene plastomers that are melt extruded into the nip between the paper and the biaxially oriented sheet. Metallocene catalyzed ethylene plastomers are preferred because they are easily melt extruded, adhere well to biaxially oriented polyolefin sheets of this invention, and adhere well to gelatin sub polyester support of this invention.

The structure of a preferred display support where the imaging layers are applied to the pigmented polyethylene is as follows:

Polyethylene layer containing  $TiO_2$

80 g/m<sup>2</sup> basis weight cellulose paper base

Metallocene catalyzed ethylene plastomer (bonding layer)

Backside biaxially oriented sheet

Conductive colloidal silica and gelatin.

The transmission display material comprising a paper base, a lower layer of biaxially oriented polymer sheet, a polyethylene layer on the upper side of said paper base, and at least one image layer overlaying said polyethylene layer wherein said polyethylene layer further comprises white pigment, optical brighteners and blue tints. The preferred white pigment is  $TiO_2$  because it enhances the sharpness of print when it is exposed by reflection. The optical brighteners provide added whiteness while the blue tints help to offset the native yellowness of gelatin which is used in imaging layers. Said polyethylene layer is further provided with an upper surface roughness of between 0.2 and 2.0

micrometers. The roughness of said surface helps to minimize glare which can distract from the message of the display material even though source of illumination is from the back.

5 The said paper base of the transmission display material comprising a paper base, a lower layer of biaxially oriented polymer sheet, a polyethylene layer on the upper side of said paper base, and at least one image layer overlaying said polyethylene layer may further comprise a white pigment to 10 tune the transmission properties of the paper base. This is important when a thin base is required and the light transmission properties need to be adjusted in order to hide the light source of the display box. In addition to controlling the transmission property of the paper base, the addition of an 15 optical brightener provides an additional appearance of whiteness to the display material. Another means to increase the transmission properties is to add polymer beads to the paper base during the formation of said base or to apply a layer of polymer beads with a binder. Said polymer beads 20 typically are hollow or have a void in the somewhat spherical structure of a particle. Such a particle or bead increases the number of air to solid interfaces which increase the opacity of the base while allowing thinner paper bases to be used. In this manner the optical properties of the paper base 25 are the predominate means of controlling the optical properties of the display material.

The transmission display material can be displayed by a method in which the display comprising a light source, and means to constrain a transmission display material in the 30 vertical and horizontal direction wherein said transmission display material comprises a paper base, a lower layer of biaxially oriented polymer sheet, a polyethylene layer on the upper side of said paper base, and at least one image layer overlaying said polyethylene layer and said light source is 35 positioned to pass light through said display material from the lower side. Such a method of display is very eye-catching and provides a very effective means grab the attention of a potential customer. The transmission of light through the image allows the image to stand out. In such as 40 display device, it is desirable not to have the light source or filaments show through the transmission display material. To provide added assurance it is desirable to have the transmission display material positioned wherein there is a gap of greater than 1 cm between the light source and the transmission display material. The gap formed in this manner is 45 desirable because it allows the light to diffuse slightly before being transmitted through the display material. This helps to prevent sharp edges of the bulbs and filament from showing through which would be very distracting for the viewer.

50 The method of forming a display material requires imaging to form an image on display material. In the case where the imaging is done with photosensitive silver halide, there is a further development step after imaging. The method of forming the display material further comprises a paper base, 55 a lower layer of biaxially oriented polymer sheet, a polyethylene layer on the upper side of said paper base, and at least one image overlaying said polyethylene layer and may further require laminating at least one sheet of environmental protection material to the transmission display material 60 and in other cases may involve laminating a sheet of environmental protection material to each side of the display material. The environmental protection material typically is a cold or hot plastic mounting material, preferably applied over the finished image. The environmental protection material is used to prevent the image or the display material from being damaged by handling or environmental conditions that 65 may be encountered when used in outdoor display applica-

tion. Display materials, as they are typically large in size, are very costly and time-consuming to make, and it is important to make sure that they are not damaged during handling or while being displayed. Environmental protection materials typically are cast or calendered vinyl, polyolefin or polyester sheets that have either a pressure sensitive adhesive or a polyethylene acrylate copolymer adhesive on one side to adhere the materials to the display material.

The sheet on the side of the base paper opposite to the imaging layers may be any suitable biaxially oriented polymer sheet. The sheet may or may not be microvoided. Bottom biaxially oriented sheets are conveniently manufactured by coextrusion of the sheet, which may contain several layers, followed by biaxial orientation. Such biaxially oriented sheets are disclosed in, for example, U.S. Pat. No. 4,764,425.

Suitable classes of thermoplastic polymers for the bottom biaxially oriented sheet core and skin layers include polyolefins, polyesters, polyamides, polycarbonates, cellulosic esters, polystyrene, polyvinyl resins, polysulfonamides, polyethers, polyimides, polyvinylidene fluoride, polyurethanes, polyphenylene sulfides, polytetrafluoroethylene, polyacetals, polysulfonates, polystyrene ionomers, and polyolefin ionomers. Copolymers and/or mixtures of these polymers can be used.

Suitable polyolefins for the core and skin layers of the bottom biaxially oriented polymer sheet include polypropylene, polyethylene, polymethylpentene, and mixtures thereof. Polyolefin copolymers, including copolymers of propylene and ethylene such as hexene, butene and octene are also useful. Polypropylenes are preferred because they are low in cost and have good strength and surface properties.

Suitable polyesters for the bottom oriented sheet include those produced from aromatic, aliphatic or cycloaliphatic dicarboxylic acids of 4-20 carbon atoms and aliphatic or alicyclic glycols having from 2-24 carbon atoms. Examples of suitable dicarboxylic acids include terephthalic, isophthalic, phthalic, naphthalene dicarboxylic acid, succinic, glutaric, adipic, azelaic, sebacic, fumaric, maleic, itaconic, 1,4-cyclohexanedicarboxylic, sodosulfoisophthalic and mixtures thereof. Examples of suitable glycols include ethylene glycol, propylene glycol, butanediol, pentanediol, hexanediol, 1,4-cyclohexanediethanol, diethylene glycol, other polyethylene glycols and mixtures thereof. Such polyesters are well known in the art and may be produced by well-known techniques, e.g., those described in U.S. Pat. No. 2,465,319 and U.S. Pat. No. 2,901,466. Preferred continuous matrix polyesters are those having repeat units from terephthalic acid or naphthalene dicarboxylic acid and at least one glycol selected from ethylene glycol, 1,4-butanediol and 1,4-cyclohexanediethanol. Poly(ethylene terephthalate), which may be modified by small amounts of other monomers, is especially preferred. Other suitable polyesters include liquid crystal copolymers formed by the inclusion of suitable amount of a co-acid component such as stilbene dicarboxylic acid. Examples of such liquid crystal copolymers are those disclosed in U.S. Pat. Nos. 4,420,607; 4,459,402; and 4,468,510.

Useful polyamides include nylon 6, nylon 66, and mixtures thereof. Copolymers of polyamides are also suitable continuous phase polymers. An example of a useful polycarbonate is bisphenol-A polycarbonate. Cellulosic esters suitable for use as the continuous phase polymer of the composite sheets include cellulose nitrate, cellulose triacetate, cellulose diacetate, cellulose acetate propionate, cellulose acetate butyrate, and mixtures or copolymers

thereof. Useful polyvinyl resins include polyvinyl chloride, poly(vinyl acetal), and mixtures thereof. Copolymers of vinyl resins can also be utilized.

The biaxially oriented sheet on the back side of the laminated base can be made with one or more layers of the same polymeric material, or it can be made with layers of different polymeric composition. In the case of a multiple layer system, when different polymeric materials are used, an additional layer may be required to promote adhesion between non-compatible polymeric materials so that the biaxially oriented sheets do not have layer fracture during manufacturing or in the final imaging element format.

The coextrusion, quenching, orienting, and heat setting of bottom biaxially oriented sheets may be effected by any process which is known in the art for producing oriented sheet, such as by a flat sheet process or a bubble or tubular process. The flat sheet process involves extruding or coextruding the blend through a slit die and rapidly quenching the extruded or coextruded web upon a chilled casting drum so that the polymer component(s) of the sheet are quenched below their solidification temperature. The quenched sheet is then biaxially oriented by stretching in mutually perpendicular directions at a temperature above the glass transition temperature of the polymer(s). The sheet may be stretched in one direction and then in a second direction or may be simultaneously stretched in both directions. After the sheet has been stretched, it is heat set by heating to a temperature sufficient to crystallize the polymers while restraining to some degree the sheet against retraction in both directions of stretching.

The surface roughness of bottom biaxially oriented sheet or  $R_a$  is a measure of relatively finely spaced surface irregularities such as those produced on the back side of photographic materials by the casting of polyethylene against a rough chilled roll. The surface roughness measurement is a measure of the maximum allowable roughness expressed in units of micrometers and by use of the symbol  $R_a$ . For the irregular profile of the back side of photographic materials of this invention, the roughness average,  $R_a$ , is the sum of the absolute value of the difference of each discrete data point from the average of all the data divided by the total number of points sampled.

Biaxially oriented polyolefin sheets commonly used in the packaging industry are commonly melt extruded and then orientated in both directions (machine direction and cross direction) to give the sheet desired mechanical strength properties. The process of biaxially orientation generally creates a surface roughness average of less than 0.23 micrometers. While a smooth surface has value in the packaging industry, use as a back side layer for photographic paper is limited. Laminated to the back side of the base paper, the biaxially oriented sheet must have a surface roughness average ( $R_a$ ) greater than 0.30 micrometers to ensure efficient transport through the many types of photofinishing equipment that have been purchased and installed around the world. At surface roughness less than 0.30 micrometers, transport through the photofinishing equipment becomes less efficient. At surface roughness greater than 2.54 micrometers, the surface would become too rough causing transport problems in photofinishing equipment and the rough back side surface would begin to emboss the silver halide emulsion as the material is wound in rolls.

The structure of a preferred backside biaxially oriented sheet utilized in the invention wherein the sheet is on the bottom of the photographic element is as follows:

Clear Polypropylene

Mixture of polypropylene and a terpolymer of ethylene-propylene-butylene (bottom).

Addenda may also be added to the biaxially oriented back side sheet to improve the whiteness of these sheets. This would include processes known in the art including adding a white pigment, such as titanium dioxide, barium sulfate, clay, or calcium carbonate. This would also include adding fluorescing agents which absorb energy in the UV region and emit light largely in the blue region, or other additives which would improve the physical properties of the sheet or the manufacturability of the sheet.

As used herein the phrase "imaging element" is a material that may be used as an imaging support for the transfer of images to the support by techniques such as ink jet printing or thermal dye transfer. Furthermore, "imaging element" may refer to a material that utilizes photosensitive silver halide in the formation of images.

The dye receiving layer or DRL for ink jet imaging may be applied by any known methods, such as solvent coating, or melt extrusion coating techniques. The DRL is coated over the tie layer or TL at a thickness ranging from 0.1–10 mm, preferably 0.5–5 mm. There are many known formulations which may be useful as dye receiving layers. The primary requirement is that the DRL is compatible with the inks which it will be imaged so as to yield the desirable color gamut and density. As the ink drops pass through the DRL, the dyes are retained or mordanted in the DRL, while the ink solvents pass freely through the DRL and are rapidly absorbed by the TL. Additionally, the DRL formulation is preferably coated from water, exhibits adequate adhesion to the TL, and allows for easy control of the surface gloss.

For example, Misuda et al in U.S. Pat. Nos. 4,879,166; 5,264,275; 5,104,730; 4,879,166; and Japanese patents 1,095,091; 2,276,671; 2,276,670; 4,267,180; 5,024,335; 5,016,517 discloses aqueous based DRL formulations comprising mixtures of psuedo-bohemite and certain water soluble resins. Light in U.S. Pat. Nos. 4,903,040; 4,930,041; 5,084,338; 5,126,194; 5,126,195; and 5,147,717, discloses aqueous-based DRL formulations comprising mixtures of vinyl pyrrolidone polymers and certain water-dispersible and/or water-soluble polyesters, along with other polymers and addenda. Butters et al in U.S. Pat. Nos. 4,857,386 and 5,102,717 discloses ink-absorbent resin layers comprising mixtures of vinyl pyrrolidone polymers and acrylic or methacrylic polymers. Sato et al. in U.S. Pat. No. 5,194,317 and Higuma et al. in U.S. Pat. No. 5,059,983 disclose aqueous-coatable DRL formulations based on poly (vinyl alcohol). Iqbal in U.S. Pat. No. 5,208,092 discloses water-based ink receiver layer or IRL formulations comprising vinyl copolymers which are subsequently cross-linked. In addition to these examples, there may be other known or contemplated DRL formulations which are consistent with the aforementioned primary and secondary requirements of the DRL, all of which fall under the spirit and scope of the current invention.

The preferred DRL is a 0.1–10 mm DRL which is coated as an aqueous dispersion of 5 parts alumoxane and 5 parts poly (vinyl pyrrolidone). The DRL may also contain varying levels and sizes of matting agents for the purpose of controlling gloss, friction, and/or fingerprint resistance, surfactants to enhance surface uniformity and to adjust the surface tension of the dried coating, mordanting agents, antioxidants, UV absorbing compounds, light stabilizers, and the like.

Although the ink-receiving elements as described above can be successfully used to achieve the objectives of the present invention, it may be desirable to overcoat the DRL for the purpose of enhancing the durability of the imaged element. Such overcoats may be applied to the DRL either

before or after the element is imaged. For example, the DRL can be overcoated with an ink-permeable layer through which inks freely pass. Layers of this type are described in U.S. Pat. Nos. 4,686,118; 5,027,131; and 5,102,717, in

5 European Patent Specification 0 524 626. Alternatively, an overcoat may be added after the element is imaged. Any of the known laminating films and equipment may be used for this purpose. The inks used in the aforementioned imaging process are well known, and the ink formulations are often closely tied to the specific processes, i.e., continuous, piezoelectric, or thermal. Therefore, depending on the specific ink process, the inks may contain widely differing amounts and combinations of solvents, colorants, preservatives, surfactants, humectants, and the like. Inks 10 preferred for use in combination with the image recording elements of the present invention are water-based, such as those currently sold for use in the Hewlett-Packard Desk Writer 560C printer. However, it is intended that alternative embodiments of the image-recording elements as described above, which may be formulated for use with inks which are specific to a given ink-recording process or to a given commercial vendor, fall within the scope of the present invention.

The thermal dye image-receiving layer of the receiving 15 elements of the invention may comprise, for example, a polycarbonate, a polyurethane, a polyester, polyvinyl chloride, poly(styrene-co-acrylonitrile), poly(caprolactone) or mixtures thereof. The dye image-receiving layer may be present in any amount which is effective for the intended purpose. In general, good results have been obtained at a concentration of from about 1 to about 10 g/m<sup>2</sup>. An overcoat layer may be further coated over the dye-receiving layer, such as described in U.S. Pat. No. 4,775,657 of Harrison et al.

20 Dye-donor elements that are used with the dye-receiving element of the invention conventionally comprise a support having thereon a dye containing layer. Any dye can be used in the dye-donor employed in the invention provided it is transferable to the dye-receiving layer by the action of heat. 25 Especially good results have been obtained with sublimable dyes. Dye donors applicable for use in the present invention are described, e.g., in U.S. Pat. Nos. 4,916,112; 4,927,803 and 5,023,228.

30 As noted above, dye-donor elements are used to form a dye transfer image. Such a process comprises image-wise-heating a dye-donor element and transferring a dye image to a dye-receiving element as described above to form the dye transfer image.

35 In a preferred embodiment of the thermal dye transfer method of printing, a dye donor element is employed which compromises a poly-(ethylene terephthalate) support coated with sequential repeating areas of cyan, magenta, and yellow dye, and the dye transfer steps are sequentially performed for each color to obtain a three-color dye transfer image. Of course, when the process is only performed for a single color, then a monochrome dye transfer image is obtained.

40 Thermal printing heads which can be used to transfer dye from dye-donor elements to receiving elements of the invention are available commercially. There can be employed, for example, a Fujitsu Thermal Head (FTP-040 MCS001), a TDK Thermal Head F415 HH7-1089 or a Rohm Thermal Head KE 2008-F3. Alternatively, other known sources of energy for thermal dye transfer may be used, such as lasers as described in, for example, GB No. 2,083,726A.

45 A thermal dye transfer assemblage of the invention comprises (a) a dye-donor element, and (b) a dye-receiving element as described above, the dye-receiving element being

in a superposed relationship with the dye-donor element so that the dye layer of the donor element is in contact with the dye image-receiving layer of the receiving element.

When a three-color image is to be obtained, the above assemblage is formed on three occasions during the time when heat is applied by the thermal printing head. After the first dye is transferred, the elements are peeled apart. A second dye-donor element (or another area of the donor element with a different dye area) is then brought in register with the dye-receiving element and the process repeated. The third color is obtained in the same manner.

The electrographic and electrophotographic processes and their individual steps have been well described in detail in many books and publications. The processes incorporate the basic steps of creating an electrostatic image, developing that image with charged, colored particles (toner), optionally transferring the resulting developed image to a secondary substrate, and fixing the image to the substrate. There are numerous variations in these processes and basic steps; the use of liquid toners in place of dry toners is simply one of those variations.

The first basic step, creation of an electrostatic image, can be accomplished by a variety of methods. The electrophotographic process of copiers uses imagewise photodischarge, through analog or digital exposure, of a uniformly charged photoconductor. The photoconductor may be a single-use system, or it may be rechargeable and reimagineable, like those based on selenium or organic photoreceptors.

In one form of the electrophotographic process of copiers uses imagewise photodischarge, through analog or digital exposure, of a uniformly charged photoconductor. The photoconductor may be a single-use system, or it may be rechargeable and reimagineable, like those based on selenium or organic photoreceptors.

In one form of the electrophotographic process, a photo-sensitive element is permanently imaged to form areas of differential conductivity. Uniform electrostatic charging, followed by differential discharge of the imaged element, creates an electrostatic image. These elements are called electrographic or xeroprinting masters because they can be repeatedly charged and developed after a single imaging exposure.

In an alternate electrographic process, electrostatic images are created iono-graphically. The latent image is created on dielectric (charge-holding) medium, either paper or film. Voltage is applied to selected metal styli or writing nibs from an array of styli spaced across the width of the medium, causing a dielectric breakdown of the air between the selected styli and the medium. Ions are created, which form the latent image on the medium.

Electrostatic images, however generated, are developed with oppositely charged toner particles. For development with liquid toners, the liquid developer is brought into direct contact with the electrostatic image. Usually a flowing liquid is employed, to ensure that sufficient toner particles are available for development. The field created by the electrostatic image causes the charged particles, suspended in a nonconductive liquid, to move by electrophoresis. The charge of the latent electrostatic image is thus neutralized by the oppositely charged particles. The theory and physics of electrophoretic development with liquid toners are well described in many books and publications.

If a reimagineable photoreceptor or an electrographic master is used, the toned image is transferred to paper (or other substrate). The paper is charged electrostatically, with the polarity chosen to cause the toner particles to transfer to the

paper. Finally, the toned image is fixed to the paper. For self-fixing toners, residual liquid is removed from the paper by air-drying or heating. Upon evaporation of the solvent these toners form a film bonded to the paper. For heat-fusible toners, thermoplastic polymers are used as part of the particle. Heating both removes residual liquid and fixes the toner to paper.

The support material of the invention preferably is coated with a silver halide photographic element capable of excellent performance when exposed by either an electronic printing method or a conventional optical printing method. An electronic printing method comprises subjecting a radiation sensitive silver halide emulsion layer of a recording element to actinic radiation of at least  $10^{-4}$  ergs/cm<sup>2</sup> for up to 100  $\mu$  seconds duration in a pixel-by-pixel mode wherein the silver halide emulsion layer is comprised of silver halide grains as described above. A conventional optical printing method comprises subjecting a radiation sensitive silver halide emulsion layer of a recording element to actinic radiation of at least  $10^{-4}$  ergs/cm<sup>2</sup> for  $10^{-3}$  to 300 seconds in an imagewise mode wherein the silver halide emulsion layer is comprised of silver halide grains as described above.

This invention in a preferred embodiment utilizes a radiation-sensitive emulsion comprised of silver halide grains (a) containing greater than 50 mole percent chloride, based on silver, (b) having greater than 50 percent of their surface area provided by {100} crystal faces, and (c) having a central portion accounting for from 95 to 99 percent of total silver and containing two dopants selected to satisfy each of the following class requirements: (i) a hexacoordination metal complex which satisfies the formula



wherein n is zero, -1, -2, -3 or -4; M is a filled frontier orbital polyvalent metal ion, other than iridium; and L<sub>6</sub> represents bridging ligands which can be independently selected, provided that least four of the ligands are anionic ligands, and at least one of the ligands is a cyano ligand or a ligand more electronegative than a cyano ligand; and (ii) an iridium coordination complex containing a thiazole or substituted thiazole ligand.

This invention is directed towards a photographic recording element comprising a support and at least one light sensitive silver halide emulsion layer comprising silver halide grains as described above.

It has been discovered quite surprisingly that the combination of dopants (i) and (ii) provides greater reduction in reciprocity law failure than can be achieved with either dopant alone. Further, unexpectedly, the combination of dopants (i) and (ii) achieve reductions in reciprocity law failure beyond the simple additive sum achieved when employing either dopant class by itself. It has not been reported or suggested prior to this invention that the combination of dopants (i) and (ii) provides greater reduction in reciprocity law failure, particularly for high intensity and short duration exposures. The combination of dopants (i) and (ii) further unexpectedly achieves high intensity reciprocity with iridium at relatively low levels, and both high and low intensity reciprocity improvements even while using conventional gelatino-peptizer (e.g., other than low methionine gelatino-peptizer).

In a preferred practical application, the advantages of the invention can be transformed into increased throughput of digital substantially artifact-free color print images while exposing each pixel sequentially in synchronism with the digital data from an image processor.

In one embodiment, the present invention represents an improvement on the electronic printing method.

Specifically, this invention in one embodiment is directed to an electronic printing method which comprises subjecting a radiation sensitive silver halide emulsion layer of a recording element to actinic radiation of at least  $10^{-4}$  ergs/cm<sup>2</sup> for up to  $100\mu$  seconds duration in a pixel-by-pixel mode. The present invention realizes an improvement in reciprocity failure by selection of the radiation sensitive silver halide emulsion layer. While certain embodiments of the invention are specifically directed towards electronic printing, use of the emulsions and elements of the invention is not limited to such specific embodiment, and it is specifically contemplated that the emulsions and elements of the invention are also well suited for conventional optical printing.

It has been unexpectedly discovered that significantly improved reciprocity performance can be obtained for silver halide grains (a) containing greater than 50 mole percent chloride, based on silver, and (b) having greater than 50 percent of their surface area provided by {100} crystal faces by employing a hexacoordination complex dopant of class (i) in combination with an iridium complex dopant comprising a thiazole or substituted thiazole ligand. The reciprocity improvement is obtained for silver halide grains employing conventional gelatino-peptizer, unlike the contrast improvement described for the combination of dopants set forth in U.S. Pat. Nos. 5,783,373 and 5,783,378, which requires the use of low methionine gelatino-peptizers as discussed therein, and which states it is preferable to limit the concentration of any gelatino-peptizer with a methionine level of greater than 30 micromoles per gram to a concentration of less than 1 percent of the total peptizer employed. Accordingly, in specific embodiments of the invention, it is specifically contemplated to use significant levels (i.e., greater than 1 weight percent of total peptizer) of conventional gelatin (e.g., gelatin having at least 30 micromoles of methionine per gram) as a gelatino-peptizer for the silver halide grains of the emulsions of the invention. In preferred embodiments of the invention, gelatino-peptizer is employed which comprises at least 50 weight percent of gelatin containing at least 30 micromoles of methionine per gram, as it is frequently desirable to limit the level of oxidized low methionine gelatin which may be used for cost and certain performance reasons.

In a specific, preferred form of the invention it is contemplated to employ a class (i) hexacoordination complex dopant satisfying the formula:



where

n is zero, -1, -2, -3, or -4;

M is a filled frontier orbital polyvalent metal ion, other than iridium, preferably  $Fe^{+2}$ ,  $Ru^{+2}$ ,  $Os^{+2}$ ,  $Co^{+3}$ ,  $Rh^{+3}$ ,  $Pd^{+4}$  or  $Pt^{+4}$ , more preferably an iron, ruthenium or osmium ion, and most preferably a ruthenium ion;

$L_6$  represents six bridging ligands which can be independently selected, provided that least four of the ligands are anionic ligands and at least one (preferably at least 3 and optimally at least 4) of the ligands is a cyano ligand or a ligand more electronegative than a cyano ligand. Any remaining ligands can be selected from among various other bridging ligands, including aquo ligands, halide ligands (specifically, fluoride, chloride, bromide and iodide), cyanate ligands, thiocyanate ligands, selenocyanate ligands, tellurocyanate ligands, and azide ligands. Hexacoordinated transition metal complexes of class (i) which include six cyano ligands are specifically preferred.

Illustrations of specifically contemplated class (i) hexacoordination complexes for inclusion in the high chloride grains are provided by Olm et al U.S. Pat. No. 5,503,970; and Daubendiek et al U.S. Pat. Nos. 5,494,789 and 5,503,971; and Keevert et al U.S. Pat. No. 4,945,035; as well as Murakami et al Japanese Patent Application Hei-2[1990]-249588, and *Research Disclosure* Item 36736. Useful neutral and anionic organic ligands for class (ii) dopant hexacoordination complexes are disclosed by Olm et al U.S. Pat. No. 5,360,712 and Kuromoto et al U.S. Pat. No. 5,462,849.

Class (i) dopant is preferably introduced into the high chloride grains after at least 50 (most preferably 75 and optimally 80) percent of the silver has been precipitated, but before precipitation of the central portion of the grains has been completed. Preferably class (i) dopant is introduced before 98 (most preferably 95 and optimally 90) percent of the silver has been precipitated. Stated in terms of the fully precipitated grain structure, class (i) dopant is preferably present in an interior shell region that surrounds at least 50 (most preferably 75 and optimally 80) percent of the silver and, with the more centrally located silver, accounts the entire central portion (99 percent of the silver), most preferably accounts for 95 percent, and optimally accounts for 90 percent of the silver halide forming the high chloride grains. The class (i) dopant can be distributed throughout the interior shell region delimited above or can be added as one or more bands within the interior shell region.

Class (i) dopant can be employed in any conventional useful concentration. A preferred concentration range is from  $10^{-8}$  to  $10^{-3}$  mole per silver mole, most preferably from  $10^{-6}$  to  $5 \times 10^{-3}$  mole per silver mole.

The following are specific illustrations of class (i) dopants:

- (i-1)  $[Fe(CN)_6]^{-4}$
- (i-2)  $[Ru(CN)_6]^{-4}$
- (i-3)  $[Os(CN)_6]^{-4}$
- (i-4)  $[Rh(CN)_6]^{-3}$
- (i-5)  $[Co(CN)_6]^{-3}$
- (i-6)  $[Fe(pyrazine)(CN)_5]^{-4}$
- (i-7)  $[RuCl(CN)_5]^{-4}$
- (i-8)  $[OsBr(CN)_5]^{-4}$
- (i-9)  $[RhF(CN)_5]^{-3}$
- (i-10)  $[In(NCS)_6]^{-3}$
- (i-11)  $[FeCO(CN)_5]^{-3}$
- (i-12)  $[RuF_2(CN)_4]^{-4}$
- (i-13)  $[OsCl_2(CN)_4]^{-4}$
- (i-14)  $[RhI_2(CN)_4]^{-3}$
- (i-15)  $[Ga(NCS)_6]^{-3}$
- (i-16)  $[Ru(CN)_5(OCN)]^{-4}$
- (i-17)  $[Ru(CN)_5(N_3)]^{-4}$
- (i-18)  $[Os(CN)_5(SCN)]^{-4}$
- (i-19)  $[Rh(CN)_5(SeCN)]^{-3}$
- (i-20)  $[Os(CN)Cl_5]^{-4}$
- (i-21)  $[Fe(CN)_3Cl_3]^{-3}$
- (i-22)  $[RU(CO)_2(CN)_4]^{-1}$

When the class (i) dopants have a net negative charge, it is appreciated that they are associated with a counter ion when added to the reaction vessel during precipitation. The counter ion is of little importance, since it is ionically dissociated from the dopant in solution and is not incorporated within the grain. Common counter ions known to be fully compatible with silver chloride precipitation, such as ammonium and alkali metal ions, are contemplated. It is

noted that the same comments apply to class (ii) dopants, otherwise described below.

The class (ii) dopant is an iridium coordination complex containing at least one thiazole or substituted thiazole ligand. Careful scientific investigations have revealed Group VIII hexahalo coordination complexes to create deep electron traps, as illustrated R. S. Eachus, R. E. Graves and M. T. Olm *J. Chem. Phys.*, Vol. 69, pp. 4580-7 (1978) and *Physica Status Solidi A*, Vol. 57, 429-37 (1980) and R. S. Eachus and M. T. Olm *Annu. Rep. Prog. Chem. Sect. C. Phys. Chem.*, Vol. 83, 3, pp. 3-48 (1986). The class (ii) dopants employed in the practice of this invention are believed to create such deep electron traps. The thiazole ligands may be substituted with any photographically acceptable substituent which does not prevent incorporation of the dopant into the silver halide grain. Exemplary substituents include lower alkyl (e.g., alkyl groups containing 1-4 carbon atoms), and specifically methyl. A specific example of a substituted thiazole ligand which may be used in accordance with the invention is 5-methylthiazole. The class (ii) dopant preferably is an iridium coordination complex having ligands each of which are more electropositive than a cyano ligand. In a specifically preferred form the remaining non-thiazole or non-substituted-thiazole ligands of the coordination complexes forming class (ii) dopants are halide ligands.

It is specifically contemplated to select class (ii) dopants from among the coordination complexes containing organic ligands disclosed by Olm et al U.S. Pat. No. 5,360,712; Olm et al U.S. Pat. No. 5,457,021; and Kuromoto et al U.S. Pat. No. 5,462,849.

In a preferred form it is contemplated to employ as a class (ii) dopant a hexacoordination complex satisfying the formula:



(II)

wherein

$n$  is zero, -1, -2, -3 or -4; and

$L_6$  represents six bridging ligands which can be independently selected, provided that at least four of the ligands are anionic ligands, each of the ligands is more electropositive than a cyano ligand, and at least one of the ligands comprises a thiazole or substituted thiazole ligand. In a specifically preferred form at least four of the ligands are halide ligands, such as chloride or bromide ligands.

Class (ii) dopant is preferably introduced into the high chloride grains after at least 50 (most preferably 85 and optimally 90) percent of the silver has been precipitated, but before precipitation of the central portion of the grains has been completed. Preferably class (ii) dopant is introduced before 99 (most preferably 97 and optimally 95) percent of the silver has been precipitated. Stated in terms of the fully precipitated grain structure, class (ii) dopant is preferably present in an interior shell region that surrounds at least 50 (most preferably 85 and optimally 90) percent of the silver and, with the more centrally located silver, accounts the entire central portion (99 percent of the silver), most preferably accounts for 97 percent, and optimally accounts for 95 percent of the silver halide forming the high chloride grains. The class (ii) dopant can be distributed throughout the interior shell region delimited above or can be added as one or more bands within the interior shell region.

Class (ii) dopant can be employed in any conventional useful concentration. A preferred concentration range is from  $10^{-9}$  to  $10^{-4}$  mole per silver mole. Iridium is most

preferably employed in a concentration range of from  $10^{-8}$  to  $10^{-5}$  mole per silver mole.

Specific illustrations of class (ii) dopants are the following:

- 5 (ii-1)  $[\text{IrCl}_5(\text{thiazole})]^{-2}$
- (ii-2)  $[\text{IrCl}_4(\text{thiazole})_2]^{-1}$
- (ii-3)  $[\text{IrBr}_5(\text{thiazole})]^{-2}$
- (ii-4)  $[\text{IrBr}_4(\text{thiazole})_2]^{-1}$
- (ii-5)  $[\text{IrCl}_5(5\text{-methylthiazole})]^{-2}$
- (ii-6)  $[\text{IrCl}_4(5\text{-methylthiazole})_2]^{-1}$
- (ii-7)  $[\text{IrBr}_5(5\text{-methylthiazole})]^{-2}$
- (ii-8)  $[\text{IrBr}_4(5\text{-methylthiazole})_2]^{-1}$ .

In one preferred aspect of the invention in a layer using a magenta dye forming coupler, a class (ii) dopant in combination with an  $\text{OsCl}_5(\text{NO})$  dopant has been found to produce a preferred result.

Emulsions demonstrating the advantages of the invention can be realized by modifying the precipitation of conventional high chloride silver halide grains having predominantly (>50%) {100} crystal faces by employing a combination of class (i) and (ii) dopants as described above.

The silver halide grains precipitated contain greater than 50 mole percent chloride, based on silver. Preferably the grains contain at least 70 mole percent chloride and, optimally at least 90 mole percent chloride, based on silver. Iodide can be present in the grains up to its solubility limit, which is in silver iodochloride grains, under typical conditions of precipitation, about 11 mole percent, based on silver. It is preferred for most photographic applications to limit iodide to less than 5 mole percent iodide, most preferably less than 2 mole percent iodide, based on silver.

Silver bromide and silver chloride are miscible in all proportions. Hence, any portion, up to 50 mole percent, of the total halide not accounted for chloride and iodide, can be bromide. For color reflection print (i.e., color paper) uses bromide is typically limited to less than 10 mole percent based on silver and iodide is limited to less than 1 mole percent based on silver.

In a widely used form high chloride grains are precipitated to form cubic grains—that is, grains having {100} major faces and edges of equal length. In practice ripening effects usually round the edges and corners of the grains to some extent. However, except under extreme ripening conditions substantially more than 50 percent of total grain surface area is accounted for by {100} crystal faces.

High chloride tetradecahedral grains are a common variant of cubic grains. These grains contain 6 {100} crystal faces and 8 {111} crystal faces. Tetradecahedral grains are within the contemplation of this invention to the extent that greater than 50 percent of total surface area is accounted for by {100} crystal faces.

Although it is common practice to avoid or minimize the incorporation of iodide into high chloride grains employed in color paper, it is has been recently observed that silver iodochloride grains with {100} crystal faces and, in some instances, one or more {111} faces offer exceptional levels of photographic speed. In these emulsions iodide is incorporated in overall concentrations of from 0.05 to 3.0 mole percent, based on silver, with the grains having a surface shell of greater than 50 Å that is substantially free of iodide and a interior shell having a maximum iodide concentration that surrounds a core accounting for at least 50 percent of total silver. Such grain structures are illustrated by Chen et al EPO 0 718 679.

In another improved form the high chloride grains can take the form of tabular grains having {100} major faces.

Preferred high chloride {100} tabular grain emulsions are those in which the tabular grains account for at least 70 (most preferably at least 90) percent of total grain projected area. Preferred high chloride {100} tabular grain emulsions have average aspect ratios of at least 5 (most preferably at least >8). Tabular grains typically have thicknesses of less than 0.3  $\mu\text{m}$ , preferably less than 0.2  $\mu\text{m}$ , and optimally less than 0.07  $\mu\text{m}$ . High chloride {100} tabular grain emulsions and their preparation are disclosed by Maskasky U.S. Pat. Nos. 5,264,337 and 5,292,632; House et al U.S. Pat. No. 5,320,938; Brust et al U.S. Pat. No. 5,314,798; and Chang et al U.S. Pat. No. 5,413,904.

Once high chloride grains having predominantly {100} crystal faces have been precipitated with a combination of class (i) and class (ii) dopants described above, chemical and spectral sensitization, followed by the addition of conventional addenda to adapt the emulsion for the imaging application of choice can take any convenient conventional form. These conventional features are illustrated by *Research Disclosure*, Item 38957, cited above, particularly:

III. Emulsion washing;

IV. Chemical sensitization;

V. Spectral sensitization and desensitization;

VII. Antifoggants and stabilizers;

VIII. Absorbing and scattering materials;

IX. Coating and physical property modifying addenda; and

X. Dye image formers and modifiers.

Some additional silver halide, typically less than 1 percent, based on total silver, can be introduced to facilitate chemical sensitization. It is also recognized that silver halide can be epitaxially deposited at selected sites on a host grain to increase its sensitivity. For example, high chloride {100} tabular grains with corner epitaxy are illustrated by Maskasky U.S. Pat. No. 5,275,930. For the purpose of providing a clear demarcation, the term "silver halide grain" is herein employed to include the silver necessary to form the grain up to the point that the final {100} crystal faces of the grain are formed. Silver halide later deposited that does not overlie the {100} crystal faces previously formed accounting for at least 50 percent of the grain surface area is excluded in determining total silver forming the silver halide grains. Thus, the silver forming selected site epitaxy is not part of the silver halide grains while silver halide that deposits and provides the final {100} crystal faces of the grains is included in the total silver forming the grains, even when it differs significantly in composition from the previously precipitated silver halide.

Image dye-forming couplers may be included in the element such as couplers that form cyan dyes upon reaction with oxidized color developing agents which are described in such representative patents and publications as: U.S. Pat. Nos. 2,367,531; 2,423,730; 2,474,293; 2,772,162; 2,895,826; 3,002,836; 3,034,892; 3,041,236; 4,883,746 and "Farbkuppler—Eine Literature Ubersicht," published in Agfa Mitteilungen, Band III, pp. 156-175 (1961). Preferably such couplers are phenols and naphthols that form cyan dyes on reaction with oxidized color developing agent. Also preferable are the cyan couplers described in, for instance, European Patent Application Nos. 491,197; 544,322; 556,700; 556,777; 565,096; 570,006; and 574,948.

Typical cyan couplers are represented by the following formulas:

CYAN-1



CYAN-2



CYAN-3



CYAN-4



wherein R<sub>1</sub>, R<sub>5</sub> and R<sub>8</sub> each represents a hydrogen or a substituent; R<sub>2</sub> represents a substituent; R<sub>3</sub>, R<sub>4</sub> and R<sub>7</sub> each represents an electron attractive group having a Hammett's substituent constant  $s_{para}$  of 0.2 or more and the sum of the  $s_{para}$  values of R<sub>3</sub> and R<sub>4</sub> is 0.65 or more; R<sub>6</sub> represents an electron attractive group having a Hammett's substituent constant  $s_{para}$  of 0.35 or more; X represents a hydrogen or a coupling-off group; Z<sub>1</sub> represents nonmetallic atoms necessary for forming a nitrogen-containing, six-membered, heterocyclic ring which has at least one dissociative group; Z<sub>2</sub> represents  $-(R_7)=$  and  $-N=$ ; and Z<sub>3</sub> and Z<sub>4</sub> each represents  $-(R_8)=$  and  $-N=$ .

For purposes of this invention, an "NB coupler" is a dye-forming coupler which is capable of coupling with the developer 4-amino-3-methyl-N-ethyl-N-(2-methanesulfonamidoethyl) aniline sesquisulfate hydrate to form a dye for which the left bandwidth (LBW) of its absorption spectra upon "spin coating" of a 3% w/v solution of the dye in di-n-butyl sebacate solvent is at least 5 nm. less than the LBW for a 3% w/v solution of the same dye in acetonitrile. The LBW of the spectral curve for a dye is the distance between the left side of the spectral curve and the wavelength of maximum absorption measured at a density of half the maximum.

The "spin coating" sample is prepared by first preparing a solution of the dye in di-n-butyl sebacate solvent (3% w/v). If the dye is insoluble, dissolution is achieved by the addition of some methylene chloride. The solution is filtered and 0.1-0.2 ml is applied to a clear polyethylene terephthalate support (approximately 4 cm x 4 cm) and spun at 4,000 RPM using the Spin Coating equipment, Model No. EC101, available from Headway Research Inc., Garland Tex. The transmission spectra of the so prepared dye samples are then recorded.

Preferred "NB couplers" form a dye which, in n-butyl sebacate, has a LBW of the absorption spectra upon "spin coating" which is at least 15 nm, preferably at least 25 nm, less than that of the same dye in a 3% solution (w/v) in acetonitrile.

In a preferred embodiment the cyan dye-forming "NB coupler" useful in the invention has the formula (IA)



(IA)

wherein

R' and R'' are substituents selected such that the coupler is a "NB coupler", as herein defined; and

Z is a hydrogen atom or a group which can be split off by the reaction of the coupler with an oxidized color developing agent.

The coupler of formula (IA) is a 2,5-diamido phenolic cyan coupler wherein the substituents R' and R'' are preferably independently selected from unsubstituted or substituted alkyl, aryl, amino, alkoxy and heterocycl groups.

In a further preferred embodiment, the "NB coupler" has the formula (I):



(I)

wherein

R'' and R''' are independently selected from unsubstituted or substituted alkyl, aryl, amino, alkoxy and heterocycl groups and Z is as hereinbefore defined;

R<sub>1</sub> and R<sub>2</sub> are independently hydrogen or an unsubstituted or substituted alkyl group; and

Typically, R'' is an alkyl, amino or aryl group, suitably a phenyl group. R''' is desirably an alkyl or aryl group or a 5-10 membered heterocyclic ring which contains one or more heteroatoms selected from nitrogen, oxygen and sulfur, which ring group is unsubstituted or substituted.

In the preferred embodiment the coupler of formula (I) is a 2,5-diamido phenol in which the 5-amido moiety is an amide of a carboxylic acid which is substituted in the alpha position by a particular sulfone ( $-\text{SO}_2^-$ ) group, such as, for example, described in U.S. Pat. No. 5,686,235. The sulfone moiety is an unsubstituted or substituted alkylsulfone or a heterocyclic sulfone or it is an arylsulfone, which is preferably substituted, in particular in the meta and/or para position.

Couplers having these structures Qf formulae (I) or (IA) comprise cyan dye-forming "NB couplers" which form image dyes having very sharp-cutting dye hues on the short wavelength side of the absorption curves with absorption maxima ( $\lambda_{max}$ ) which are shifted hypsochromically and are generally in the range of 620-645 nm, which is ideally suited for producing excellent color reproduction and high color saturation in color photographic papers.

Referring to formula (I), R<sub>1</sub> and R<sub>2</sub> are independently hydrogen or an unsubstituted or substituted alkyl group,

preferably having from 1 to 24 carbon atoms and in particular 1 to 10 carbon atoms, suitably a methyl, ethyl, n-propyl, isopropyl, butyl or decyl group or an alkyl group substituted with one or more fluoro, chloro or bromo atoms, such as a trifluoromethyl group. Suitably, at least one of R<sub>1</sub> and R<sub>2</sub> is a hydrogen atom and if only one of R<sub>1</sub> and R<sub>2</sub> is a hydrogen atom then the other is preferably an alkyl group having 1 to 4 carbon atoms, more preferably one to three carbon atoms and desirably two carbon atoms.

As used herein and throughout the specification unless where specifically stated otherwise, the term "alkyl" refers to an unsaturated or saturated straight or branched chain alkyl group, including alkenyl, and includes aralkyl and cyclic alkyl groups, including cycloalkenyl, having 3-8 carbon atoms and the term 'aryl' includes specifically fused aryl.

In formula (I), R'' is suitably an unsubstituted or substituted amino, alkyl or aryl group or a 5-10 membered heterocyclic ring which contains one or more heteroatoms selected from nitrogen, oxygen and sulfur, which ring is unsubstituted or substituted, but is more suitably an unsubstituted or substituted phenyl group.

Examples of suitable substituent groups for this aryl or heterocyclic ring include cyano, chloro, fluoro, bromo, iodo, alkyl- or aryl-carbonyl, alkyl- or aryl-oxycarbonyl, carbonamido, alkyl- or aryl-carbonamido, alkyl- or aryl-sulfonyl, alkyl- or aryl-sulfonyloxy, alkyl- or aryl-oxysulfonyl, alkyl- or aryl-sulfoxide, alkyl- or aryl-sulfamoyl, alkyl- or aryl-sulfonamido, aryl, alkyl, alkoxy, aryloxy, nitro, alkyl- or aryl-ureido and alkyl- or aryl-carbamoyl groups, any of which may be further substituted. Preferred groups are halogen, cyano, alkoxy carbonyl, alkylsulfamoyl, alkyl-sulfonamido, alkylsulfonyl, carbamoyl, alkylcarbamoyl or alkylcarbonamido. Suitably, R'' is a 4-chlorophenyl, 3,4-di-chlorophenyl, 3,4-difluorophenyl, 4-cyanophenyl, 3-chloro-4-cyanophenyl, pentafluorophenyl, or a 3- or 4-sulfonamidophenyl group.

In formula (I), when R''' is alkyl it may be unsubstituted or substituted with a substituent such as halogen or alkoxy.

When R''' is aryl or a heterocycle, it may be substituted. Desirably, it is not substituted in the position alpha to the sulfonyl group.

In formula (I), when R''' is a phenyl group, it may be substituted in the meta and/or para positions with one to three substituents independently selected from the group consisting of halogen, and unsubstituted or substituted alkyl, alkoxy, aryloxy, acyloxy, acylamino, alkyl- or aryl-sulfonyloxy, alkyl- or aryl-sulfamoyl, alkyl- or aryl-sulfamoyl amino, alkyl- or aryl-sulfonamido, alkyl- or aryl-ureido, alkyl- or aryl-oxycarbonyl, alkyl- or aryl-oxy-carbamoyl and alkyl- or aryl-carbamoyl groups.

In particular, each substituent may be an alkyl group such as methyl, t-butyl, heptyl, dodecyl, pentadecyl, octadecyl or 1,1,2,2-tetramethylpropyl; an alkoxy group such as methoxy, t-butoxy, octyloxy, dodecyloxy, tetradecyloxy, hexadecyloxy or octadecyloxy; an aryloxy group such as phenoxy, 4-t-butylphenoxy or 4-dodecyl-phenoxy; an alkyl- or aryl-acyloxy group such as acetoxy or dodecanoyloxy; an alkyl- or aryl-acylamino group such as acetamido, hexadecanamido or benzamido; an alkyl- or aryl-sulfonyloxy group such as methyl-sulfonyloxy, dodecylsulfonyloxy or 4-methylphenyl-sulfonyloxy; an alkyl- or aryl-sulfamoyl group such as N-butylsulfamoyl or N-4-t-butylphenylsulfamoyl; an alkyl- or aryl-sulfamoyl amino group such as N-butyl-sulfamoyl amino or N-4-t-butylphenylsulfamoyl-amino; an alkyl- or aryl-sulfonamido group such as methane-sulfonamido, hexadecanesulfona-

25

mido or 4-chlorophenyl-sulfonamido; an alkyl- or arylureido group such as methylureido or phenylureido; an alkoxy- or aryloxy-carbonyl such as methoxycarbonyl or phenoxy carbonyl; an alkoxy- or aryloxy-carbonylamino group such as methoxy-carbonylamino or phenoxy carbonylamino; an alkyl- or aryl-carbamoyl group such as N-butylcarbamoyl or N-methyl-N-dodecylcarbamoyl; or a perfluoroalkyl group such as trifluoromethyl or heptafluoropropyl.

Suitably the above substituent groups have 1 to 30 carbon atoms, more preferably 8 to 20 aliphatic carbon atoms. A desirable substituent is an alkyl group of 12 to 18 aliphatic carbon atoms such as dodecyl, pentadecyl or octadecyl or an alkoxy group with 8 to 18 aliphatic carbon atoms such as dodecyloxy and hexadecyoxy or a halogen such as a meta or para chloro group, carboxy or sulfonamido. Any such groups may contain interrupting heteroatoms such as oxygen to form e.g. polyalkylene oxides.

In formula (I) or (IA) Z is a hydrogen atom or a group which can be split off by the reaction of the coupler with an oxidized color developing agent, known in the photographic art as a 'coupling-off group' and may preferably be hydrogen, chloro, fluoro, substituted aryloxy or mercaptotetrazole, more preferably hydrogen or chloro.

The presence or absence of such groups determines the chemical equivalency of the coupler, i.e., whether it is a 2-equivalent or 4-equivalent coupler, and its particular identity can modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation, color correction, and the like.

Representative classes of such coupling-off groups include, for example, halogen, alkoxy, aryloxy, heterocyclyloxy, sulfonyloxy, acyloxy, acyl, heterocyclsulfonamido, heterocyclthio, benzothiazolyl, phosphonyloxy, alkylthio, arylthio, and arylazo. These coupling-off groups are described in the art, for example, in U.S. Pat. Nos. 2,455,169; 3,227,551; 3,432,521; 3,467,563; 3,617,291; 3,880,661; 4,052,212; and 4,134,766; and in U.K. Patent Nos. and published applications 1,466,728; 1,531,927; 1,533,039; 2,066,755A, and 2,017,704A. Halogen, alkoxy and aryloxy groups are most suitable.

Examples of specific coupling-off groups are —Cl, —F, —Br, —SCN, —OCH<sub>3</sub>, —OC<sub>6</sub>H<sub>5</sub>, —OCH<sub>2</sub>C(=O)NHCH<sub>2</sub>CH<sub>2</sub>OH, —OCH<sub>2</sub>C(O)NHCH<sub>2</sub>CH<sub>2</sub>OCH<sub>3</sub>, —OCH<sub>2</sub>C(O)NHCH<sub>2</sub>CH<sub>2</sub>OC(=O)OCH<sub>3</sub>, —P(=O)(OC<sub>2</sub>H<sub>5</sub>)<sub>2</sub>, —SCH<sub>2</sub>CH<sub>2</sub>COOH,



26

-continued



Typically, the coupling-off group is a chlorine atom, hydrogen atom or p-methoxyphenoxy group.

It is essential that the substituent groups be selected so as to adequately ballast the coupler and the resulting dye in the organic solvent in which the coupler is dispersed. The ballasting may be accomplished by providing hydrophobic substituent groups in one or more of the substituent groups. Generally a ballast group is an organic radical of such size and configuration as to confer on the coupler molecule sufficient bulk and aqueous insolubility as to render the coupler substantially nondiffusible from the layer in which it is coated in a photographic element. Thus, the combination of substituent are suitably chosen to meet these criteria. To be effective, the ballast will usually contain at least 8 carbon atoms and typically contains 10 to 30 carbon atoms. Suitable ballasting may also be accomplished by providing a plurality of groups which in combination meet these criteria. In the preferred embodiments of the invention R<sub>1</sub> in formula (I) is a small alkyl group or hydrogen. Therefore, in these embodiments the ballast would be primarily located as part of the other groups. Furthermore, even if the coupling-off group Z contains a ballast it is often necessary to ballast the other substituents as well, since Z is eliminated from the molecule upon coupling; thus, the ballast is most advantageously provided as part of groups other than Z.

The following examples further illustrate preferred coupler of the invention. It is not to be construed that the present invention is limited to these examples.

27



IC-1



IC-2



IC-3



IC-4

28

-continued

IC-5



60

65

29

-continued



IC-9

5

10



IC-10



30

40



IC-12 45



-continued

IC-13



IC-15



IC-16



**31**

-continued



IC-17

5



IC-18

10



IC-19

15



20



IC-20

25



30



35

35



40

40

45

45

50

50

55

55

60

60

65

**32**

-continued

IC-21

IC-22

IC-23

IC-24

**33**

-continued

IC-25



IC-26



IC-27



IC-28



IC-29

**34**

-continued

IC-29



IC-30



IC-31



**35**

-continued

**36**

-continued

IC-37



60 Preferred couplers are IC-3, IC-7, IC-35, and IC-36 because of their suitably narrow left bandwidths.

65 Couplers that form magenta dyes upon reaction with oxidized color developing agent are described in such representative patents and publications as: U.S. Pat. Nos. 2,311,

082; 2,343,703; 2,369,489; 2,600,788; 2,908,573; 3,062, 5 653; 3,152,896; 3,519,429; 3,758,309; and "Farbkuppler-eine Literature Ubersicht," published in Agfa Mitteilungen, Band III, pp. 126-156 (1961). Preferably, such couplers are pyrazolones, pyrazolotriazoles, or pyrazolobenzimidazoles that form magenta dyes upon reaction with oxidized color 10 developing agents. Especially preferred couplers are 1H-pyrazolo [5,1-c]-1,2,4-triazole and 1H-pyrazolo [1,5-b]-1,2,4-triazole. Examples of 1H-pyrazolo [5,1-c]-1,2,4-triazole couplers are described in U.K. Patent Nos. 1,247, 15 493; 1,252,418; 1,398,979; U.S. Pat. Nos. 4,443,536; 4,514, 490; 4,540,654; 4,590,153; 4,665,015; 4,822,730; 4,945, 034; 5,017,465; and 5,023,170. Examples of 1H-pyrazolo [1,5-b]-1,2,4-triazoles can be found in European Patent 20 176,804; 177,765; U.S Patent Nos. 4,659,652; 5,066,575; and 5,250,400.

Typical pyrazoloazole and pyrazolone couplers are represented by the following formulas:



MAGENTA-1



MAGENTA-2

wherein  $R_a$  and  $R_b$  independently represent H or a substituent;  $R_c$  is a substituent (preferably an aryl group);  $R_d$  is a substituent (preferably an anilino, carbonamido, ureido, carbamoyl, alkoxy, aryloxycarbonyl, alkoxy carbonyl, or N-heterocyclic group);  $X$  is hydrogen or a coupling-off group; and  $Z_a$ ,  $Z_b$ , and  $Z_c$  are independently a substituted methine group,  $=N-$ ,  $=C-$ , or  $-NH-$ , provided that one of either the  $Z_a-Z_b$  bond or the  $Z_b-Z_c$  bond is a double bond and the other is a single bond, and when the  $Z_b-Z_c$  bond is a carbon-carbon double bond, it may form part of an aromatic ring, and at least one of  $Z_a$ ,  $Z_b$ , and  $Z_c$  represents a methine group connected to the group  $R_b$ .

Specific examples of such couplers are:



M-1

-continued

M-2



M-3



M-4



M-5



Couplers that form yellow dyes upon reaction with oxidized color developing agent are described in such representative patents and publications as: U.S. Pat. Nos. 2,298, 50 443; 2,407,210; 2,875,057; 3,048,194; 3,265,506; 3,447, 928; 3,960,570; 4,022,620; 4,443,536; 4,910,126; and 5,340,703 and "Farbkuppler-eine Literature Ubersicht," published in Agfa Mitteilungen, Band III, pp. 112-126 (1961). Such couplers are typically open chain ketomethylene compounds. Also preferred are yellow couplers such as described in, for example, European Patent Application Nos. 482,552; 510,535; 524,540; 543,367; and U.S. Pat. No. 60 5,238,803. For improved color reproduction, couplers which give yellow dyes that cut off sharply on the long wavelength side are particularly preferred (for example, see U.S. Pat. No. 5,360,713).

65 Typical preferred yellow couplers are represented by the following formulas:



wherein R<sub>1</sub>, R<sub>2</sub>, Q<sub>1</sub> and Q<sub>2</sub> each represents a substituent; X is hydrogen or a coupling-off group; Y represents an aryl group or a heterocyclic group; Q<sub>3</sub> represents an organic residue required to form a nitrogen-containing heterocyclic group together with the >N—; and Q<sub>4</sub> represents nonmetallic atoms necessary to from a 3- to 5-membered hydrocarbon ring or a 3- to 5-membered heterocyclic ring which contains at least one hetero atom selected from N, O, S, and P in the ring. Particularly preferred is when Q<sub>1</sub> and Q<sub>2</sub> each represent an alkyl group, an aryl group, or a heterocyclic group, and R<sub>2</sub> represents an aryl or tertiary alkyl group.

30  
35  
40  
45  
50

5  
10  
15  
20  
25



Y-4  
20  
25



Y-1  
45  
50  
55  
60  
65



Unless otherwise specifically stated, substituent groups 55 which may be substituted on molecules herein include any groups, whether substituted or unsubstituted, which do not 55 destroy properties necessary for photographic utility. When the term "group" is applied to the identification of a substituent containing a substitutable hydrogen, it is intended to 60 encompass not only the substituent's unsubstituted form, but also its form further substituted with any group or groups as herein mentioned. Suitably, the group may be halogen or may be bonded to the remainder of the molecule by an atom of carbon, silicon, oxygen, nitrogen, phosphorous, or sulfur. 65 The substituent may be, for example, halogen, such as chlorine, bromine or fluorine; nitro; hydroxyl; cyano; carboxyl; or groups which may be further substituted, such as

41

alkyl, including straight or branched chain alkyl, such as methyl, trifluoromethyl, ethyl, t-butyl, 3-(2,4-di-t-pentylphenoxy) propyl, and tetradecyl; alkenyl, such as ethylene, 2-butene; alkoxy, such as methoxy, ethoxy, propoxy, butoxy, 2-methoxyethoxy, sec-butoxy, hexyloxy, 2-ethylhexyloxy, tetradecyloxy, 2-(2,4-di-t-pentylphenoxy) ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthoxy, and 4-tolyloxy; carbonamido, such as acetamido, benzamido, butyramido, tetradecanamido, alpha-(2,4-di-t-pentyl-phenoxy)acetamido, alpha-(2,4-di-t-pentylphenoxy) butyramido, alpha-(3-pentadecylphenoxy)-hexanamido, alpha-(4-hydroxy-3-t-butylphenoxy)-tetradecanamido, 10 2-oxo-pyrrolidin-1-yl, 2-oxo-5-tetradecylpyrrolin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, phenoxy carbonylamino, benzoyloxycarbonylamino, hexadecyloxycarbonylamino, 20 2,4-di-t-butylphenoxy carbonylamino, phenylcarbonylamino, 2,5-(di-t-pentylphenyl) carbonylamino, p-dodecyl-phenylcarbonylamino, p-tolylcarbonylamino, N-methylureido, N,N-dimethylureido, N-methyl-N-dodecylureido, 25 N-hexadecylureido, N,N-dioctadecylureido, N,N-diethyl-N'-ethylureido, N-phenylureido, N,N-diphenylureido, N-phenyl-N-p-tolylureido, N-(m-hexadecylphenyl)ureido, N,N-(2,5-di-t-pentylphenyl)-N'-ethylureido, and t-butylcarbonamido; sulfonamido, such as 30 methylsulfonamido, benzenesulfonamido, p-tolylsulfonamido, p-dodecylbenzenesulfonamido, N-methyltetradecylsulfonamido, N,N-dipropylsulfamoyl, and hexadecylsulfonamido; sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecyloxy)propyl]sulfamoyl, N-[4-(2,4-di-t-pentylphenoxy)butyl]sulfamoyl, N-methyl-N-tetradecylsulfamoyl, and N-dodecylsulfamoyl; carbamoyl, such as N-methylcarbamoyl, N,N-dibutylcarbamoyl, N-octadecylcarbamoyl, N-[4-(2,4-di-t-pentylphenoxy)butyl]carbamoyl, N-methyl-N-tetradecylcarbamoyl, and N,N-dioctylcarbamoyl; acyl, such as acetyl, (2,4-di-t-amylphenoxy)acetyl, phenoxy carbonyl, p-dodecyloxyphenoxy carbonyl, methoxycarbonyl, 45 butoxycarbonyl, tetradecyloxycarbonyl, ethoxycarbonyl, benzoyloxycarbonyl, 3-pentadecyloxycarbonyl, and dodecyloxycarbonyl; sulfonyl, such as methoxysulfonyl, octyloxy sulfonyl, tetradecyloxy sulfonyl, 2-ethylhexyloxy sulfonyl, phenoxy sulfonyl, 2,4-di-t-pentylphenoxy sulfonyl, methylsulfonyl, octylsulfonyl, 50 2-ethylhexylsulfonyl, dodecylsulfonyl, hexadecylsulfonyl, phenylsulfonyl, 4-nonylphenylsulfonyl, and p-tolylsulfonyl; sulfonyloxy, such as dodecylsulfonyloxy, and hexadecylsulfonyloxy; sulfinyl, such as methylsulfinyl, octylsulfinyl, 55 2-ethylhexylsulfinyl, dodecylsulfinyl, hexadecylsulfinyl, phenylsulfinyl, 4-nonylphenylsulfinyl, and p-tolylsulfinyl; thio, such as ethylthio, octylthio, benzylthio, tetradecylthio, 2-(2,4-di-t-pentylphenoxy) ethylthio, phenylthio, 2-butoxy-5-t-octylphenylthio, and p-tolylthio; acyloxy, such as acetoxy, benzoyloxy, octadecanoyloxy, p-dodecylamidobenzoyloxy, N-phenylcarbamoyloxy, N-ethylcarbamoyloxy, and cyclohexylcarbonyloxy; amino, such as phenylanilino, 60 2-chloroanilino, diethylamino, dodecylamino; imino, such as 1 (N-phenylimido)ethyl, N-succinimido or 3-benzylhydantoinyl; phosphate, such as dimethylphosphate

42

and ethylbutylphosphate; phosphite, such as diethyl and dihexylphosphite; a heterocyclic group, a heterocyclic oxy group or a heterocyclic thio group, each of which may be substituted and which contain a 3 to 7 membered heterocyclic ring composed of carbon atoms and at least one hetero atom selected from the group consisting of oxygen, nitrogen and sulfur, such as 2-furyl, 2-thienyl, 2-benzimidazolyl or 2-benzothiazolyl; quaternary ammonium, such as triethylammonium; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups, etc. Generally, the above groups and substituents thereof may include those having up to 48 carbon atoms, typically 1 to 36 carbon atoms and usually less than 24 carbon atoms, but greater numbers are possible depending on the particular substituents selected.

Representative substituents on ballast groups include alkyl, aryl, alkoxy, aryloxy, alkylthio, hydroxy, halogen, alkoxy carbonyl, arylox carbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 42 carbon atoms. Such substituents can also be further substituted.

Stabilizers and scavengers that can be used in these photographic elements, but are not limited to, the following.

ST-1



ST-2



ST-3



ST-4



**43**

-continued

**44**

-continued

ST-5



ST-6



ST-7



ST-8



ST-9



ST-10



ST-11

ST-12

ST-13

ST-14

ST-15

ST-16

**45**

-continued

**46**

-continued

ST-24



Examples of solvents which may be used in the invention include the following:

|                                                 |      |
|-------------------------------------------------|------|
| Tritolyl phosphate                              | S-1  |
| Dibutyl phthalate                               | S-2  |
| Diundecyl phthalate                             | S-3  |
| N,N-Diethyldecanamide                           | S-4  |
| N,N-Dibutyldecanamide                           | S-5  |
| Tris(2-ethylhexyl)phosphate                     | S-6  |
| Acetyl tributyl citrate                         | S-7  |
| 2,4-Di-tert-pentylphenol                        | S-8  |
| 2-(2-Butoxyethoxy)ethyl acetate                 | S-9  |
| 1,4-Cyclohexyldimethylene bis(2-ethylhexanoate) | S-10 |

The dispersions used in photographic elements may also include ultraviolet (UV) stabilizers and so-called liquid UV stabilizers such as described in U.S. Pat. Nos. 4,992,358; 4,975,360; and 4,587,346. Examples of UV stabilizers are shown below.



n:m 1:1 mw = 75-100,000

-continued



The aqueous phase may include surfactants. Surfactant may be cationic, anionic, zwitterionic or non-ionic. Useful 60 surfactants include, but are not limited to, the following:



Further, it is contemplated to stabilize photographic dispersions prone to particle growth through the use of hydrophobic, photographically inert compounds such as disclosed by Zengerle et al in U.S. Pat. No. 5,468,604.

In a preferred embodiment the invention employs recording elements which are constructed to contain at least three silver halide emulsion layer units. A suitable full color, multilayer format for a recording element used in the invention is represented by Structure I.

| STRUCTURE I                                                               |  |
|---------------------------------------------------------------------------|--|
| Red-sensitized<br>cyan dye image-forming silver halide emulsion unit      |  |
| Interlayer                                                                |  |
| Green-sensitized<br>magenta dye image-forming silver halide emulsion unit |  |
| Interlayer                                                                |  |
| Blue-sensitized<br>yellow dye image-forming silver halide emulsion unit   |  |
| //// Support ////                                                         |  |

#### STRUCTURE I

wherein the red-sensitized, cyan dye image-forming silver halide emulsion unit is situated nearest the support; next in order is the green-sensitized, magenta dye image-forming unit, followed by the uppermost blue-sensitized, yellow dye image-forming unit. The image-forming units are separated from each other by hydrophilic colloid interlayers containing an oxidized developing agent scavenger to prevent color contamination. Silver halide emulsions satisfying the grain and gelatino-peptizer requirements described above can be present in any one or combination of the emulsion layer units. Additional useful multicolor, multilayer formats for an element of the invention include structures as described in U.S. Pat. No. 5,783,373. Each of such structures in accordance with the invention preferably would contain at least three silver halide emulsions comprised of high chloride grains having at least 50 percent of their surface area bounded by {100} crystal faces and containing dopants from classes (i) and (ii), as described above. Preferably each of the emulsion layer units contains emulsion satisfying these criteria.

Conventional features that can be incorporated into multilayer (and particularly multicolor) recording elements contemplated for use in the method of the invention are illustrated by *Research Disclosure*, Item 38957, cited above:

#### XI. Layers and layer arrangements

#### XII. Features applicable only to color negative

#### XIII. Features applicable only to color positive

#### B. Color reversal

#### C. Color positives derived from color negatives

#### XIV. Scan facilitating features.

The recording elements comprising the radiation sensitive high chloride emulsion layers according to this invention can be conventionally optically printed, or in accordance with a particular embodiment of the invention can be image-wise exposed in a pixel-by-pixel mode using suitable high energy radiation sources typically employed in electronic printing methods. Suitable actinic forms of energy encompass the ultraviolet, visible and infrared regions of the electromagnetic spectrum as well as electron-beam radiation and is conveniently supplied by beams from one or more light emitting diodes or lasers, including gaseous or solid state lasers. Exposures can be monochromatic, orthochromatic or panchromatic. For example, when the recording element is a multilayer multicolor element, exposure can be provided by laser or light emitting diode beams of appropriate spectral radiation, for example, infrared, red, green or blue wavelengths, to which such element is sensitive. Multicolor elements can be employed which produce cyan, magenta and yellow dyes as a function of exposure in separate portions of the electromagnetic spectrum, including at least two portions of the infrared region, as disclosed in the previously mentioned U.S. Pat. No. 4,619,892. Suitable exposures include those up to 2000 nm, preferably up to 1500 nm. Suitable light emitting diodes and commercially available laser sources are known and commercially available. Imagewise exposures at ambient, elevated or reduced temperatures and/or pressures can be employed within the useful response range of the recording element determined by conventional sensitometric techniques, as illustrated by T. H. James, *The Theory of the Photographic Process*, 4th Ed., Macmillan, 1977, Chapters 4, 6, 17, 18 and 23.

It has been observed that anionic  $[MX_xY_yL_z]$  hexacoordination complexes, where M is a group 8 or 9 metal (preferably iron, ruthenium or iridium), X is halide or pseudohalide (preferably Cl, Br or CN) x is 3 to 5, Y is  $H_2O$ , y is 0 or 1, L is a C—C, H—C or C—N—H organic ligand, and Z is 1 or 2, are surprisingly effective in reducing high intensity reciprocity failure (HIRF), low intensity reciprocity failure (LIRF) and thermal sensitivity variance and in improving latent image keeping (LIK). As herein employed HIRF is a measure of the variance of photographic properties for equal exposures, but with exposure times ranging from  $10^{-1}$  to  $10^{-6}$  second. LIRF is a measure of the variance of photographic properties for equal exposures, but with exposure times ranging from  $10^{-1}$  to 100 seconds. Although these advantages can be generally compatible with face centered cubic lattice grain structures, the most striking improvements have been observed in high (>50 mole %, preferably >90 mole %) chloride emulsions. Preferred C—C, H—C or C—N—H organic ligands are aromatic heterocycles of the type described in U.S. Pat. No. 5,462,849. The most effective C—C, H—C or C—N—H organic ligands are azoles and azines, either unsubstituted or containing alkyl, alkoxy or halide substituents, where the alkyl moieties contain from 1 to 8 carbon atoms. Particularly preferred azoles and azines include thiazoles, thiazolines and pyrazines.

The quantity or level of high energy actinic radiation provided to the recording medium by the exposure source is generally at least  $10^{-4}$  ergs/cm<sup>2</sup>, typically in the range of about  $10^{-4}$  ergs/cm<sup>2</sup> to  $10^{-3}$  ergs/cm<sup>2</sup> and often from  $10^{-3}$  ergs/cm<sup>2</sup> to  $10^2$  ergs/cm<sup>2</sup>. Exposure of the recording element in a pixel-by-pixel mode as known in the prior art persists for only a very short duration or time. Typical maximum exposure times are up to 100  $\mu$  seconds, often up to 10  $\mu$

seconds, and frequently up to only  $0.5 \mu$  seconds. Single or multiple exposures of each pixel are contemplated. The pixel density is subject to wide variation, as is obvious to those skilled in the art. The higher the pixel density, the sharper the images can be, but at the expense of equipment complexity. In general, pixel densities used in conventional electronic printing methods of the type described herein do not exceed  $10^7$  pixels/cm<sup>2</sup> and are typically in the range of about  $10^4$  to  $10^6$  pixels/cm<sup>2</sup>. An assessment of the technology of high-quality, continuous-tone, color electronic printing using silver halide photographic paper which discusses various features and components of the system, including exposure source, exposure time, exposure level and pixel density and other recording element characteristics is provided in Firth et al., *A Continuous-Tone Laser Color Printer*, Journal of Imaging Technology, Vol. 14, No. 3, June 1988, which is hereby incorporated herein by reference. As previously indicated herein, a description of some of the details of conventional electronic printing methods comprising scanning a recording element with high energy beams such as light emitting diodes or laser beams, are set forth in Hioki U.S. Pat. No. 5,126,235; European Patent Applications 479 167 Al and 502 508 A1.

Once imagewise exposed, the recording elements can be processed in any convenient conventional manner to obtain a viewable image. Such processing is illustrated by *Research Disclosure*, Item 38957, cited above:

#### XVIII. Chemical development systems

#### XIX. Development

#### XX. Desilvering, washing, rinsing and stabilizing.

In addition, a useful developer for the inventive material is a homogeneous, single part developing agent. The homogeneous, single-part color developing concentrate is prepared using a critical sequence of steps:

In the first step, an aqueous solution of a suitable color developing agent is prepared. This color developing agent is generally in the form of a sulfate salt. Other components of the solution can include an antioxidant for the color developing agent, a suitable number of alkali metal ions (in an at least stoichiometric proportion to the sulfate ions) provided by an alkali metal base, and a photographically inactive water-miscible or water-soluble hydroxy-containing organic solvent. This solvent is present in the final concentrate at a concentration such that the weight ratio of water to the organic solvent is from about 15:85 to about 50:50.

In this environment, especially at high alkalinity, alkali metal ions and sulfate ions form a sulfate salt that is precipitated in the presence of the hydroxy-containing organic solvent. The precipitated sulfate salt can then be readily removed using any suitable liquid/solid phase separation technique (including filtration, centrifugation or decantation). If the antioxidant is a liquid organic compound, two phases may be formed and the precipitate may be removed by discarding the aqueous phase.

The color developing concentrates of this invention include one or more color developing agents that are well known in the art that, in oxidized form, will react with dye forming color couplers in the processed materials. Such color developing agents include, but are not limited to, aminophenols, p-phenylenediamines (especially N,N-dialkyl-p-phenylenediamines) and others which are well known in the art, such as EP 0 434 097A1 (published Jun. 26, 1991) and EP 0 530 921A1 (published Mar. 10, 1993). It may be useful for the color developing agents to have one or more water-solubilizing groups as are known in the art.

Further details of such materials are provided in *Research Disclosure*, publication 38957, pages 592-639 (September

1996). *Research Disclosure* is a publication of Kenneth Mason Publications Ltd., Dudley House, 12 North Street, Emsworth, Hampshire PO10 7DQ England (also available from Emsworth Design Inc., 121 West 19th Street, New York, N.Y. 10011). This reference will be referred to hereinafter as "Research Disclosure".

Preferred color developing agents include, but are not limited to, N,N-diethyl p-phenylenediamine sulfate (KODAK Color Developing Agent CD-2), 4-amino-3-methyl-N-(2-methane sulfonamidoethyl)aniline sulfate, 4-(N-ethyl-N-b-hydroxyethylamino)-2-methylaniline sulfate (KODAK Color Developing Agent CD-4), p-hydroxyethylaminoaniline sulfate, 4-(N-ethyl-N-2-methanesulfonylaminooethyl)-2-methylphenylenediamine sesquisulfate (KODAK Color Developing Agent CD-3), 4-(N-ethyl-N-2-methanesulfonylaminooethyl)-2-methylphenylenediamine sesquisulfate, and others readily apparent to one skilled in the art.

In order to protect the color developing agents from oxidation, one or more antioxidants are generally included 20 in the color developing compositions. Either inorganic or organic antioxidants can be used. Many classes of useful antioxidants are known, including but not limited to, sulfites (such as sodium sulfite, potassium sulfite, sodium bisulfite and potassium metabisulfite), hydroxylamine (and derivatives thereof), hydrazines, hydrazides, amino acids, ascorbic acid (and derivatives thereof), hydroxamic acids, aminoketones, mono- and polysaccharides, mono- and polyamines, quaternary ammonium salts, nitroxy radicals, alcohols, and oximes. Also useful as antioxidants are 1,4-cyclohexadienes. Mixtures of compounds from the same or 25 different classes of antioxidants can also be used if desired.

Especially useful antioxidants are hydroxylamine derivatives as described for example, in U.S. Pat. Nos. 4,892,804; 4,876,174; 5,354,646; and 5,660,974, all noted above, and U.S. Pat. No. 5,646,327 (Burns et al). Many of these 30 antioxidants are mono- and dialkylhydroxylamines having one or more substituents on one or both alkyl groups. Particularly useful alkyl substituents include sulfo, carboxy, amino, sulfonamido, carbonamido, hydroxy and other solubilizing substituents.

More preferably, the noted hydroxylamine derivatives can be mono- or dialkylhydroxylamines having one or more hydroxy substituents on the one or more alkyl groups. Representative compounds of this type are described for example in U.S. Pat. No. 5,709,982 (Marrese et al) as having the structure I:



50 wherein R is hydrogen, a substituted or unsubstituted alkyl group of 1 to 10 carbon atoms, a substituted or unsubstituted hydroxyalkyl group of 1 to 10 carbon atoms, a substituted or unsubstituted cycloalkyl group of 5 to 10 carbon atoms, or a substituted or unsubstituted aryl group having 6 to 10 carbon atoms in the aromatic nucleus.

55 X<sub>1</sub> is —CR<sub>2</sub>(OH)CHR<sub>1</sub>— and X<sub>2</sub> is —CH<sub>2</sub>CR<sub>1</sub>(OH)R— where R<sub>1</sub> and R<sub>2</sub> are independently hydrogen, hydroxy, a substituted or unsubstituted alkyl group or 1 or 2 carbon atoms, a substituted or unsubstituted hydroxyalkyl group of 1 or 2 carbon atoms, or R<sub>1</sub> and R<sub>2</sub> together represent the carbon atoms necessary to complete a substituted or unsubstituted 5- to 8-membered saturated or unsaturated carbocyclic ring structure.

60 Y is a substituted or unsubstituted alkylene group having at least 4 carbon atoms, and has an even number of carbon

atoms, or Y is a substituted or unsubstituted divalent aliphatic group having an even total number of carbon and oxygen atoms in the chain, provided that the aliphatic group has a least 4 atoms in the chain.

Also in Structure I, m, n and p are independently 0 or 1. Preferably, each of m and n is 1, and p is 0.

Specific di-substituted hydroxylamine antioxidants include, but are not limited to: N,N-bis(2,3-dihydroxypropyl)hydroxylamine, N,N-bis(2-methyl-2,3-dihydroxypropyl)hydroxylamine and N,N-bis(1-hydroxymethyl-2-hydroxy-3-phenylpropyl)hydroxylamine. The first compound is preferred.

The following examples illustrate the practice of this invention. They are not intended to be exhaustive of all possible variations of the invention. Parts and percentages are by weight unless otherwise indicated.

## EXAMPLES

### Example 1

In this example a low cost paper based transmission display material utilizing a biaxially oriented polymer sheet laminated to the back side of the support was compared to a typical polyester based transmission display product. This example will show that the low cost transmission display material provides an superior image as the density minimum areas of the images were substantially neutral compared to the yellow minimum areas for the control. Further, several advantages for the low cost paper base material will be obvious.

#### Control:

The control sample utilized in this invention was a commercial available display material. The control material was a typical pigmented polyester base material coated with a light sensitized silver halide emulsion.

The paper utilized in the invention is as follows:

The cellulose paper base was produced by refining a pulp furnish of 50% bleached hardwood kraft, 25% bleached hardwood sulfite, and 25% bleached softwood sulfite through a double disk refiner, then a Jordan conical refiner to a Canadian Standard Freeness of 200 cc. To the resulting pulp furnish was added 0.2% alkyl ketene dimer, 1.0% cationic cornstarch, 0.5% polyamide-epichlorohydrin, 0.26 anionic polyacrylamide, and 5.0% TiO<sub>2</sub> on a dry weight basis. A 70 g/m<sup>2</sup> bone dry weight base paper was made on a fourdrinier paper machine, wet pressed to a solid of 42%, and dried to a moisture of 10% using steam-heated dryers achieving a Sheffield Porosity of 160 Sheffield Units and an apparent density 0.70 g/cc. The paper base was then surface sized using a vertical size press with a 10% hydroxyethylated cornstarch solution to achieve a loading of 3.3 wt. % starch. The surface sized support was calendered to an apparent density of 1.04 gm/cc.

The above paper base was backside laminated with a oriented polyolefin sheet that contained a rough skin layer for machine transport. The above paper base was melt extrusion coated with low density polyethylene containing anatase TiO<sub>2</sub> for whiteness and sharpness on the top side. The structure of the invention is as follows:

12 g/m<sup>2</sup> low density polyethylene with 12% anatase TiO<sub>2</sub>

Cellulose grade paper of the example

12 g/m<sup>2</sup> 70% low density polyethylene/30% ethylene plastomer

Biaxially oriented polypropylene

Polyethylene with a terpolymer of ethylene-propylene-butylene

Antistatic layer consisting of colloid silica and acrylate binder.

The invention support material was coated with a digitally working light sensitive silver halide emulsion. The emulsion was applied to the melt cast polyethylene layer.

| Layer      | Item                                                                        | Laydown (g/m <sup>2</sup> ) |
|------------|-----------------------------------------------------------------------------|-----------------------------|
| 10 Layer 1 | <u>Blue Sensitive Layer</u>                                                 |                             |
| 20         | Gelatin                                                                     | 1.3127                      |
|            | Blue sensitive silver (Blue EM-1)                                           | 0.2399                      |
|            | Y-4                                                                         | 0.4143                      |
|            | ST-23                                                                       | 0.4842                      |
|            | Tributyl Citrate                                                            | 0.2179                      |
|            | ST-24                                                                       | 0.1211                      |
|            | ST-16                                                                       | 0.0095                      |
|            | Sodium Phenylmercaptotetrazole                                              | 0.0001                      |
|            | Piperidino hexose reductone                                                 | 0.0024                      |
|            | 5-chloro-2-methyl-4-isothiazolin-3-one/ 2-methyl-4-isothiazolin-3-one (3/1) | 0.0002                      |
|            | SF-1                                                                        | 0.0366                      |
|            | Potassium chloride                                                          | 0.0204                      |
|            | Dye-1                                                                       | 0.0148                      |
| 25 Layer 2 | <u>Interlayer</u>                                                           |                             |
| 30         | Gelatin                                                                     | 0.7532                      |
|            | ST-4                                                                        | 0.1076                      |
|            | S-3                                                                         | 0.1969                      |
|            | 5-chloro-2-methyl-4-isothiazolin-3-one/ 2-methyl-4-isothiazolin-3-one (3/1) | 0.0000                      |
|            | Catechol disulfonate                                                        | 0.0323                      |
|            | SF-1                                                                        | 0.0081                      |
| 35 Layer 3 | <u>Green Sensitive Layer</u>                                                |                             |
| 40         | Gelatin                                                                     | 1.1944                      |
|            | Green Sensitive silver (Green EM-1)                                         | 0.1011                      |
|            | M-4                                                                         | 0.2077                      |
|            | Oleyl Alcohol                                                               | 0.2174                      |
|            | S-3                                                                         | 0.1119                      |
|            | ST-21                                                                       | 0.0398                      |
|            | ST-22                                                                       | 0.2841                      |
|            | Dye-2                                                                       | 0.0073                      |
|            | 5-chloro-2-methyl-4-isothiazolin-3-one/ 2-methyl-4-isothiazolin-3-one (3/1) | 0.0001                      |
|            | SF-1                                                                        | 0.0236                      |
|            | Potassium chloride                                                          | 0.0204                      |
|            | Sodium Phenylmercaptotetrazole                                              | 0.0007                      |
| 45 Layer 4 | <u>M/C Interlayer</u>                                                       | 0.0000                      |
| 50         | Gelatin                                                                     | 0.7532                      |
|            | ST-4                                                                        | 0.1076                      |
|            | S-3                                                                         | 0.1969                      |
|            | Acrylamide/t-Butylacrylamide sulfonate copolymer                            | 0.0541                      |
|            | Bis-vinylsulfonylmethane                                                    | 0.1390                      |
|            | 3,5-Dinitrobenzoic acid                                                     | 0.0000                      |
|            | Citric acid                                                                 | 0.0007                      |
|            | Catechol disulfonate                                                        | 0.0323                      |
|            | 5-chloro-2-methyl-4-isothiazolin-3-one/ 2-methyl-4-isothiazolin-3-one (3/1) | 0.0000                      |
| 55 Layer 5 | <u>Red Sensitive Layer</u>                                                  | 0.0000                      |
| 60         | Gelatin                                                                     | 1.3558                      |
|            | Red Sensitive silver (Red EM-1)                                             | 0.1883                      |
|            | IC-35                                                                       | 0.2324                      |
|            | IC-36                                                                       | 0.0258                      |

The display material was processed as a minimum density. The display support was measured for status A density using an X-Rite Model 310 photographic densitometer. Spectral transmission is calculated from the Status A density readings and is the ratio of the transmitted power to the incident power and is expressed as a percentage as follows;

$T_{RGB}=10^{-D} \cdot 100$  where D is the average of the red, green, and blue Status A transmission density response. The display material was also measured for L\*, a\*, and b\* using a Spectrogard spectrophotometer, CIE system, using illuminant D6500. In the transmission mode, a qualitative assessment was made as to the amount of illuminating backlighting show through. A substantial amount of show through would be considered undesirable as the nonfluorescent light sources could interfere with the image quality. The comparison data for invention and control are listed in Table 1 below.

TABLE 1

| Parameter              | Invention | Control |
|------------------------|-----------|---------|
| % Transmission         | 40%       | 51%     |
| Backlight Show through | None      | Slight  |
| CIE D6500 b*           | -1.1      | 10.5    |
| CIE D6500 a*           | -0.71     | -0.62   |
| CIE D6500 L*           | 85        | 71      |

The transmission display material of this invention is clearly is superior to prior art transmission display material. It is lighter and whiter in appearance while providing improved opacity to minimize show through. For transmission display materials, a bluer white is more perceptually preferred than yellow whites. The invention is considerably more blue as indicated by a -1.1 as compared to 10.5. Furthermore, the use of the paper base to diffuse the transmission light source provided a superior diffusion screen as opposed to the use of expensive  $TiO_2$  in the control display material control. Because the invention utilized a thin cellulose paper base to both diffuse the illuminating light source and provide stiffness for efficient transport in photographic printing and development equipment, the invention is lower in cost compared to the control material. Finally, because a cast polyethylene surface was utilized on the top size, the light sensitive silver halide emulsion layer had acceptable adhesion without the need for expensive primers. In addition to the emulsion adhesion, the cast polyethylene layer can be used to provide a rough, nonglossy surface that would avoid the need for post process application of a matte coating.

The invention has been described in detail with particular reference to certain preferred embodiments thereof, but it will be understood that variations and modifications can be effected within the spirit and scope of the invention.

What is claimed is:

1. A transmission display material comprising a paper base, a lower layer of biaxially oriented polymer sheet, a polyethylene layer on the upper side of said paper base, and at least one image layer overlaying said polyethylene layer.
2. The material of claim 1 wherein said image layer comprises at least one silver halide containing layer.
3. The material of claim 1 wherein said image layer comprises at least one ink jet receiving layer or thermal dye transfer receiving layer.
4. The material of claim 1 wherein said material has a percent spectral transmission of between 30 and 70 percent.
5. The material of claim 1 wherein said material has a percent spectral transmission of between 40 and 60 percent.
6. The material of claim 1 wherein said paper base has a basis weight of between 50 and 150 g/m<sup>2</sup>.
7. The display material of claim 1 wherein said material has a tensile strength of greater than 17,000 kPa in the machine direction and 13,600 kPa in the cross direction.

8. The display material of claim 1 wherein said material has a tensile strength of between 20,400 kPa and 68,000 kPa in both the machine and cross direction.

9. The display material of claim 1 wherein said polymer sheet is transparent.

10. The display material of claim 1 wherein said polymer sheet has a bottom surface roughness of between 0.2 and 0.8  $\mu m$ .

11. The display material of claim 1 wherein said polymer sheet comprises a polyolefin polymer.

12. The display material of claim 1 wherein said polymer sheet comprises polypropylene.

13. The material of claim 1 wherein said paper base has a basis weight of between 50 and 150 g/m<sup>2</sup> and an apparent density of between 0.97 and 1.2 g/cc.

14. The material of claim 13 wherein said paper further comprises a white pigment.

15. The material of claim 1 wherein said paper further comprises an optical brightener.

16. The material of claim 1 wherein said polyethylene layer further comprises white pigment, optical brightener, and blue tints.

17. The material of claim 1 wherein said polyethylene layer is provided with an upper surface roughness of between 0.2 and 2.0  $\mu m$ .

18. The material of claim 1 wherein the back surface of said material is provided with an antistat layer.

19. The material of claim 1 wherein said paper further comprises voided polymer beads.

20. A method of display comprising a light source and means to constrain a transmission display material in the vertical and horizontal direction wherein said transmission display material comprises a paper base, a lower layer of biaxially oriented polymer sheet, a polyethylene layer on the upper side of said paper base, and at least one image layer overlaying said polyethylene layer and said light source is positioned to pass light through said display material from the lower side.

21. The method of claim 20 wherein there is provided a gap of greater than 1 centimeter between said light source and said transmission display material.

22. A method of forming a display material comprising providing a transmission display material comprising a paper base, a lower layer of biaxially oriented polymer sheet, a polyethylene layer on the upper side of said paper base, and at least one image layer overlaying said polyethylene layer, imaging said transmission display material, laminating at least one sheet of environmental protection material to said transmission display material.

23. The method of claim 22 wherein a sheet of environmental protection material is laminated to each side of said transmission display material.

24. The method of claim 22 wherein said image layer comprises photosensitive silver halide and the method further comprises developing after said imaging and before laminating.